# EUROPEAN PATENT APPLICATION

(11) **EP 4 685 260 A1**
(43) Date of publication of application: **28.01.2026**
(21) Application number: 24810653.6
(22) Date of filing: 27.02.2024
(51) Int. Cl.: C22C 38/00, C21D 9/46, C22C 38/14, C22C 38/60

(54) **HIGH-STRENGTH STEEL SHEET AND METHOD FOR PRODUCING SAME**

(30) Priority: 19.05.2023 JP 2023082882
(71) Applicant: JFE Steel Corporation, Tokyo, 100-0011 (JP)
(72) Inventor: MORIMOTO, Ryohei, Tokyo 100-0011 (JP); ENDOH, Kazuki, Tokyo 100-0011 (JP); TADA, Masaki, Tokyo 100-0011 (JP); NISHIYAMA, Takeshi, Tokyo 100-0011 (JP)
(74) Representative: Hoffmann Eitle
(86) International application number: PCT/JP2024/007146
(87) International publication number: WO 2024/241645

(57) **Abstract**

The present invention is directed to providing a steel sheet having excellent LME resistance, high strength, and good formability by a method different from conventional techniques, and to providing a method for manufacturing the steel sheet.

A high-strength steel sheet containing particular components and having a particular microstructure, wherein the relationship between the amount of dissolved Nb (Nbₛₒₗ), the amount of Nb in Nb precipitates having a particle size of less than 20 nm (Nbₚᵣₑ), and the total amount of Nb contained in the steel sheet (Nb) satisfies the following Formula 1, and wherein the amount of diffusible hydrogen in the steel is 0.50 mass ppm or less: $\left({Nb}_{sol}/Nb\right) + \left({Nb}_{pre}/Nb\right) \geq 0.40$ where Nbₛₒₗ represents the amount (mass %) of dissolved Nb, and Nbₚᵣₑ represents the amount (mass %) of Nb in Nb precipitates having a particle size of less than 20 nm.

## Description

### Technical Field

The present invention relates to a steel sheet and a method for manufacturing the same. In particular, the present invention relates to a high-strength steel sheet having excellent LME resistance, which is suitable as a member to be subjected to forming by cold pressing for use in an industrial field such as the automotive industry and the electrical machinery industry, and to a method for manufacturing the steel sheet.

### Background Art

In recent years, from the viewpoint of global environmental protection, there has been an increasing need for weight reduction of car bodies to improve fuel efficiency. Therefore, the use of high-strength steel sheets for automotive parts is desired. When cold-rolled steel sheets are used for automotive parts, a method is generally used in which two or more steel sheets, which have undergone a forming process, are joined by welding and finished into a desired shape.

In the production of automotive parts, spot welding is mainly used to join steel sheets together. It is known that when welding is performed on a sheet assembly including a high-strength steel sheet (high-strength galvanized steel sheet) having a welded galvanizing layer, cracking is likely to occur in a weld.

This is considered to be due to the fact that a galvanized coating layer, which generally has a low melting point, will liquefy during welding and penetrate into grain boundaries in the base steel sheet, causing a reduction in the grain boundary strength. Such a reduction in strength due to liquefied metal is generally called liquid metal embrittlement (LME). Cracking that occurs due to liquid metal embrittlement is called liquid metal embrittlement (LME) cracking.

It is also known that cracking occurs in a weld even in a high-strength steel sheet having no coating when a mating material to which the high-strength steel sheet is welded has a galvanized coating layer. Such LME cracking that occurs in a high-strength steel sheet having no coating layer is herein referred to as non-self-derived LME cracking.

The non-self-derived LME cracking is particularly noticeable when spot welding is performed with electrodes inclined at an angle. The phrase "with electrodes inclined at an angle" herein refers to a state of welding electrodes in which the axis of the electrodes is not perpendicular to the surfaces of steel sheets.

Various studies have been conducted to prevent LME cracking in a galvanized steel sheet and non-self-derived LME cracking in a non-coated steel sheet upon spot welding of the steel sheets.

For example, Patent Literature 1 discloses a technique which involves controlling the frequency of corresponding grain boundaries in the surface of a steel sheet after a high-temperature tensile test and the thickness of a softened surface region, thereby achieving a high-strength steel sheet having a tensile strength of 980 MPa or more and a total elongation of 20% or more, and having excellent LME resistance.

Patent Literature 2 discloses a technique which involves introducing oxygen into the surface of a steel slab during continuous casting, thereby forming an iron oxide as a site for the formation of titanium nitride. This inhibits B in the steel from binding to dissolved nitrogen in a later annealing process and promotes the formation of (Fe,Mn)₂B in a surface region of a steel sheet, thereby achieving a steel sheet having an LME resistance, high strength, and excellent ductility.

Patent Literature 3 proposes a technique which involves removing, prior to spot welding, a coating layer from a portion to be welded so as to prevent LME cracking.

### Citation List

### Patent Literature

PTL 1: International Publication No. WO 2020/184154
PTL 2: International Publication No. WO 2020/225936
PTL 3: International Publication No. WO 2016/159169

### Summary of Invention

### Technical Problem

However, the technique described in Patent Literature 1 necessitates a reduction in the amount of Si in order to reduce the frequency of corresponding grain boundaries in the surface of a steel sheet. It therefore appears difficult to impart good formability to a steel sheet having a strength of 980 MPa or higher grade.

Regarding the technique described in Patent Literature 2 which involves introducing oxygen into the surface of a steel slab during continuous casting to improve the LME resistance of the steel sheet finally obtained, it is expected that the introduction of oxygen into the surface of a slab will cause the formation of scale, resulting in a reduction in yield. Further, the presence of a large amount of hard particles (Fe,Mn)₂B in a surface region from the casting stage will cause surface cracking during casting.

The technique described in Patent Literature 3 requires a step of removing a coating layer in advance, which increases the production cost. Further, the removal of the coating layer will cause a reduction in the corrosion resistance of a weld.

It is therefore an object of the present invention to provide a steel sheet having excellent LME resistance, high strength, and good formability by a method different from the conventional techniques, and to provide a method for manufacturing the steel sheet. Examples of the steel sheet include a hot-rolled steel sheet, a cold-rolled steel sheet, and a coated steel sheet such as GA or GI.

In the present invention, "high strength" refers to a TS of 980 MPa or more, and "good formability" means that the relationship between tensile strength TS and elongation El, shown in the following formula 7, is satisfied. ${TS}^{1.5} \times El \geq 390000$

### Solution to Problem

In order to solve the above problems, the present inventors conducted intensive studies on the chemical compositions and microstructures of steel sheets. They have now found the following facts through precise control of slab heating conditions, temperatures from hot rolling to coiling, and annealing conditions, and through control of the states of elements existing in the steel.

By dissolving Nb or by controlling the particle radius of precipitates within a particular range which will not cause cracking on a steel surface during casting, a dissolved element which is present in the steel during welding or a dissolved element produced by dissolution of the precipitates prevents penetration of zinc into the steel, thereby improving the LME resistance. On the other hand, when the radius of precipitates of a particular element is larger than a predetermined value, the precipitates will not be dissolved sufficiently during welding, resulting in a failure to achieve an improvement in LME resistance by the dissolved element. In addition, it is quite likely that cracking will newly occur starting from coarse precipitates not only during a manufacturing process but after press forming or during welding.

The present invention is based on the above findings, and is summarized as follows.
[1] A high-strength steel sheet having a chemical composition containing, in mass %:
   C: not less than 0.030% and not more than 0.500%,
   Si: more than 0.01% and not more than 2.50%,
   Mn: not less than 0.10% and not more than 5.00%,
   P: 0.100% or less,
   S: 0.0200% or less,
   Al: 0.100% or less,
   N: 0.0100% or less,
   O: 0.0100% or less,
   Ti: not less than 0.010% and not more than 0.200%, and
   Nb: not less than 0.005% and not more than 0.500%,
   with the balance being Fe and incidental impurities,
      wherein in the microstructure of the steel sheet at a 1/4 thickness position,
      the total area fraction of tempered martensite and bainite is not less than 40% and not more than 85%,
      the area fraction of fresh martensite is not less than 0% and not more than 25%,
      the area fraction of retained austenite is not less than 5% and not more than 20%, and
      the balance includes at least one of ferrite and pearlite at an area fraction of not less than 0% and not more than 20%,
      wherein the relationship between the amount of dissolved Nb (Nbₛₒₗ), the amount of Nb in Nb precipitates having a particle size of less than 20 nm (Nbₚᵣₑ), and the total amount of Nb contained in the steel sheet (Nb) satisfies the following Formula 1, and
      wherein the amount of diffusible hydrogen in the steel is 0.50 mass ppm or less: $\left({Nb}_{sol}/Nb\right) + \left({Nb}_{pre}/Nb\right) \geq 0.40$ where Nbₛₒₗ represents the amount (mass %) of dissolved Nb, and Nbₚᵣₑ represents the amount (mass %) of Nb in Nb precipitates having a particle size of less than 20 nm.
[2] The high-strength steel sheet according to [1], wherein the chemical composition further contains, in mass %, one or two or more selected from the following:
   V: 0.500% or less,
   Ta: 0.10% or less,
   W: 0.10% or less,
   B: 0.0100% or less,
   Cr: 1.00% or less,
   Mo: 1.00% or less,
   Co: 1.00% or less,
   Ni: 1.00% or less,
   Cu: 1.00% or less,
   Sn: 0.200% or less,
   Sb: 0.200% or less,
   Ca: 0.0100% or less,
   Mg: 0.0100% or less,
   REM: 0.0100% or less,
   Zr: 0.100% or less,
   Te: 0.100% or less,
   Hf: 0.10% or less, and
   Bi: 0.200% or less.
[3] The high-strength steel sheet according to [1] or [2], having a coating layer on the surface of the steel sheet.
[4] The high-strength steel sheet according to [3], wherein the coating layer is an alloyed coating layer.
[5] A method for manufacturing the high-strength steel sheet according to [1] or [2], including:
   a slab heating step of heating a steel material having the chemical composition at a temperature equal to or higher than Tₛₒₗ°C represented by the following Formula 2 for 1.0 hours or more;
   a hot rolling step;
   a coiling step at a coiling temperature T_{CT}°C of 650°C or lower; and
   an annealing step of heating a steel sheet to a soaking temperature T_{AT}°C, holding the steel sheet at the soaking temperature T_{AT}°C of not less than 750°C and not more than 950°C, and then cooling the steel sheet,
   wherein Q_{HR} defined by Formula 3 in terms of a finish rolling start temperature T_{FET}°C, a finish rolling delivery temperature T_{FDT}°C, and an effective time t_{HR} from the start of finish rolling to the end of finish rolling in the hot rolling step,
   Q_{CT} defined by Formula 4 in terms of a residence time t_{CT} from T_{FDT}°C to 650°C and the coiling temperature T_{CT}°C in the coiling step, and
   Q_{AT} defined by Formula 5 in terms of the soaking temperature T_{AT}°C, a heating time t from 650°C to the soaking temperature T_{AT}°C, and a holding time t_{AT} at the soaking temperature T_{AT}°C in the annealing step, satisfy Formula 6:${T}_{sol} = 7900 / \left(3.42-\left(log\left(\left[Nb%\right]\left[C%\right]\right)\right)\right) - 273$ where [Nb%] and [C%] respectively represent the Nb content (mass %) and the C content (mass %) of the steel; ${Q}_{HR} = 0.5 \left({T}_{FET}+{T}_{FDT}\right) \times {log}_{10} \left({t}_{HR}\right) ;$ ${Q}_{CT} = 0.5 \left({T}_{CT}+650\right) \times {log}_{10} \left({t}_{CT}\right) ;$ QAT = 0.5(650 + TAT) × log10(t) + TAT × log10(tAT); ${Q}_{HR} + {Q}_{CT} + {Q}_{AT} \leq 6000 .$
[6] The method for manufacturing a high-strength steel sheet according to [5], wherein the value of Q_{AT} is 4700 or less.
[7] The method for manufacturing a high-strength steel sheet according to [5] or [6], wherein the steel sheet after the annealing step is subjected to a coating treatment.
[8] The method for manufacturing a high-strength steel sheet according to [7], wherein the coating treatment is an alloying coating treatment.

### Advantageous Effects of Invention

According to the present invention, it is possible to obtain a high-strength steel sheet having good formability and excellent LME resistance. Therefore, the present invention is very useful in the industrial fields of automobiles, electrical devices, etc., and is particularly useful for reducing the weight of automotive body frame parts.

### Description of Embodiments

The present invention will now be described in detail. In the following description of component elements, "%" refers to "mass %" unless otherwise specified.

(1) The following are the reasons for the above-described limitations on the chemical composition of the steel of the present invention.

### C: not less than 0.030% and not more than 0.500%

C is an element necessary for increasing the strengths of tempered martensite, bainite, and fresh martensite. In order to fully achieve this effect, it is necessary to make the C content at least 0.030%. Therefore, the C content is made 0.030% or more. The C content is preferably 0.050% or more, more preferably 0.070% or more, even more preferably 0.090% or more, and most preferably 0.100% or more. On the other hand, if the C content exceeds 0.500%, the weldability and the LME resistance of the steel, which are important in joining automotive parts, will deteriorate. Therefore, the C content is made 0.500% or less. The C content is preferably 0.400% or less, more preferably 0.300% or less, even more preferably 0.270% or less, and most preferably 0.250% or less.

### Si: more than 0.01% and not more than 2.50%

Si is an element that prevents excessive formation and growth of carbides in the steel, thereby increases the fraction of retained austenite and improving ductility. If the Si content is 0.01% or less, this effect is poor and the steel cannot have good formability. Therefore, the lower limit of the Si content is made 0.01%. The Si content is made more than 0.01%. The Si content is preferably 0.05% or more, more preferably 0.10% or more, even more preferably 0.50% or more, and most preferably 0.90% or more. However, if the Si content exceeds 2.50%, it causes a decrease in the melting point of zinc, which facilitates penetration of zinc into the steel sheet during welding, resulting in a reduction in the LME resistance of the steel sheet. Therefore, the Si content is made 2.50% or less. The Si content is preferably 2.30% or less, more preferably 2.00% or less, even more preferably 1.80% or less, and most preferably 1.60% or less.

### Mn: not less than 0.10% and not more than 5.00%

Mn is an element that affects the area fractions of tempered martensite, bainite, and fresh martensite through enhancement of hardenability. If the Mn content is less than 0.10%, a soft phase such as ferrite will be formed excessively, and desired area fractions of tempered martensite, bainite, and fresh martensite cannot be obtained, resulting in an insufficient steel sheet strength. Therefore, the Mn content is made 0.10% or more. The Mn content is preferably 0.50% or more, more preferably 0.80% or more, even more preferably 1.00% or more, and most preferably 2.00% or more. On the other hand, if the Mn content exceeds 5.00%, the ductility of the steel deteriorates due to increase in the area fractions of tempered martensite, bainite, and fresh martensite. Therefore, the Mn content is made 5.00% or less. The Mn content is preferably 4.50% or less, more preferably 4.00% or less, even more preferably 3.70% or less, and most preferably 3.50% or less.

### P: 0.100% or less

It is possible that P, through its segregation at grain boundaries and consequential embrittlement of the grain boundaries, may adversely affect the LME resistance; therefore, the P content needs to be 0.100% or less. Thus, the P content is made 0.100% or less. The P content is preferably made 0.080% or less, more preferably 0.070% or less, even more preferably 0.050% or less, and most preferably 0.040% or less.

While the lower limit of the P content is not particularly limited, in view of the fact that P is a solid solution strengthening element and can increase the strength of the steel sheet, the P content is preferably made 0.001% or more, more preferably 0.003% or more, and even more preferably 0.005% or more.

### S: 0.0200% or less

It is possible that S, through its segregation at grain boundaries and consequential embrittlement of the steel upon hot processing, and through the formation of sulfides, may adversely affect the LME resistance; therefore, the S content needs to be 0.0200% or less. Thus, the S content is made 0.0200% or less. The S content is preferably made 0.0180% or less, more preferably 0.0150% or less, even more preferably 0.0100% or less, and most preferably 0.0050% or less. While the lower limit of the S content is not particularly limited, in view of the restrictions of production technology, the S content is preferably 0.0001% or more, more preferably 0.0005% or more, and even more preferably 0.0010% or more.

### Al: 0.100% or less

Al is an element which acts as a deoxidizer and is effective in reducing inclusions in the steel, and is preferably added in a deoxidization process. On the other hand, Al increases the transformation temperature for austenitizing, resulting in inclusion of ferrite in the microstructure. Therefore, the use of Al in an amount of more than 0.100% makes it difficult to achieve a desired TS. Thus, the Al content is made 0.100% or less. The Al content is preferably made 0.080% or less, more preferably 0.070% or less, even more preferably 0.060% or less, and most preferably 0.050% or less. While the lower limit of the Al content is not particularly limited, the Al content is preferably made 0.001% or more, more preferably 0.010% or more, and even more preferably 0.020% or more.

### N: 0.0100% or less

N may adversely affect the LME resistance through the formation of coarse nitrides. If the N content exceeds 0.0100%, a large amount of coarse nitrides will be formed, leading to a significant deterioration of LME resistance. The N content is preferably as small as possible. Thus, the N content is made 0.0100% or less. The N content is preferably 0.0090% or less, more preferably 0.0080% or less, even more preferably 0.0070% or less, and most preferably 0.0060% or less. While the lower limit of the N content is not particularly limited, in view of the restrictions of production technology, the N content is preferably made 0.0001% or more, more preferably 0.0010% or more, and even more preferably 0.0020% or more.

### O: 0.0100% or less

O exists as an oxide and reduces the ductility of the steel sheet. Therefore, the O content needs to be 0.0100% or less. Thus, the O content is made 0.0100% or less. The O content is preferably 0.0075% or less, more preferably 0.0060% or less, even more preferably 0.0050% or less, and most preferably 0.0045% or less. While the lower limit of the O content is not particularly specified, in view of the restrictions of production technology, the O content is preferably made 0.0001% or more, more preferably 0.0005% or more, and even more preferably 0.0010% or more.

### Ti: not less than 0.010% and not more than 0.200%

Ti contributes to precipitation strengthening and, in addition, reduces the prior austenite grain size and thereby reduces the grain sizes of tempered martensite and bainite. Thus, Ti is effective in increasing the strength of the steel. In order to fully achieve this effect, the Ti content is made 0.010% or more. The Ti content is preferably 0.012% or more, more preferably 0.015% or more, even more preferably 0.020% or more, and most preferably 0.025% or more. However, if the Ti content exceeds 0.200%, Ti may remain undissolved during heating of the steel material before hot rolling, resulting in an increase in the amount of coarse precipitates and a reduction in ductility. Therefore, the Ti content is made 0.200% or less. The Ti content is preferably 0.180% or less, more preferably 0.150% or less, even more preferably 0.100% or less, and most preferably 0.050% or less.

### Nb: not less than 0.005% and not more than 0.500%

Nb is an element that improves the LME resistance. In particular, the presence of dissolved Nb in the steel during welding has a great effect on the improvement of the LME resistance. More specifically, by dissolving Nb or by controlling the particle radius of Nb precipitates within a particular range, the dissolved element which is present in the steel during welding or the dissolved element produced by dissolution of the precipitates prevents the penetration of zinc into the steel, thereby improving the LME resistance. In order to fully achieve such an effect, the Nb content needs to be 0.005% or more. The Nb content is preferably 0.007% or more, more preferably 0.008% or more, even more preferably 0.010% or more, and most preferably 0.012% or more. On the other hand, if the Nb content exceeds 0.500%, precipitates such as Nb carbide and Nb nitride are formed coarsely, and the precipitates are not dissolved sufficiently during welding. Therefore, the improvement of LME resistance by the dissolved element cannot be expected. Furthermore, the El of the steel sheet will be insufficient for the TS of the steel sheet. It is quite conceivable that this may cause the occurrence of new cracking starting from coarse precipitates not only during a manufacturing process but after press forming or during welding. Therefore, the Nb content is made 0.500% or less. The Nb content is preferably made 0.400% or less, more preferably 0.350% or less, even more preferably 0.200% or less, and most preferably 0.100% or less.

A high-strength steel sheet according to an embodiment of the present invention has a chemical composition containing the above-described components, with the balance including Fe and incidental impurities. Preferably, a high-strength steel sheet according to an embodiment of the present invention has a chemical composition containing the above-described components, with the balance consisting of Fe and incidental impurities. Examples of the incidental impurities may include Zn, Pb, and As. Such impurities are allowed to be present in the steel in a total amount of up to 0.100%.

In addition to the above-described components, the chemical composition may contain, in mass %, one or two or more selected from the following: V: 0.500% or less, Ta: 0.10% or less, W: 0.10% or less, B: 0.0100% or less, Cr: 1.00% or less, Mo: 1.00% or less, Co: 1.00% or less, Ni: 1.00% or less, Cu: 1.00% or less, Sn: 0.200% or less, Sb: 0.200% or less, Ca: 0.0100% or less, Mg: 0.0100% or less, REM: 0.0100% or less, Zr: 0.100% or less, Te: 0.100% or less, Hf: 0.10% or less, and Bi: 0.200% or less.

### V: 0.500% or less

V contributes to precipitation strengthening and, in addition, reduces the prior austenite grain size and thereby reduces the grain sizes of tempered martensite and bainite. Thus, V is effective in increasing the strength of the steel. The steel can therefore contain V as necessary. While the lower limit of the V content is not particularly limited, in order to achieve the above effect, the V content is preferably made 0.001% or more, more preferably 0.005% or more, and even more preferably 0.010% or more. However, if the V content exceeds 0.500%, V may remain undissolved during heating of the steel material before hot rolling, resulting in an increase in the amount of coarse precipitates and a reduction in ductility. Therefore, when the steel contains V, the V content is made 0.500% or less. The V content is preferably 0.400% or less, more preferably 0.300% or less, even more preferably 0.200% or less, and most preferably 0.100% or less.

### Ta: 0.10% or less

Ta, like Ti, contributes to increasing the strength of the steel through the formation of an alloy carbide and an alloy carbonitride. In addition, Ta partly dissolves in Nb carbide or Nb carbonitride to form a complex precipitate such as (Nb,Ta) (C,N), thereby significantly suppressing coarsening of precipitates and stabilizing the contribution of precipitation strengthening to the increase of the strength. The steel can therefore contain Ta as necessary. While the lower limit of the Ta content is not particularly limited, in order to achieve the above effect, the Ta content is preferably made 0.01% or more, more preferably 0.02% or more, and even more preferably 0.03% or more. However, a too-high Ta content will lead to saturation of the precipitate stabilizing effect and increased alloying cost. Therefore, when the steel contains Ta, the Ta content is made 0.10% or less. The Ta content is preferably made 0.08% or less, more preferably 0.07% or less, even more preferably 0.06% or less, and most preferably 0.05% or less.

### W: 0.10% or less

The steel can contain W as necessary to improve the hardenability of the steel and to further increase the strength of the steel through a reduction in the grain sizes of tempered martensite and bainite. While the lower limit of the W content is not particularly limited, in order to achieve the above effects, the W content is preferably made 0.01% or more, more preferably 0.02% or more, and even more preferably 0.03% or more. However, a W content of more than 0.10% may increase the amount of coarse precipitates, such as WN and WS, which remain undissolved during heating of the slab in a hot rolling process, resulting in a reduction in ductility. Therefore, when the steel contains W, the W content is made 0.10% or less. The W content is preferably made 0.08% or less, more preferably 0.07% or less, even more preferably 0.06% or less, and most preferably 0.05% or less.

### B: 0.0100% or less

B is an element which, through its segregation at austenite grain boundaries, can improve hardenability. B can form a microstructure composed mainly of tempered martensite and bainite, thereby increasing the strength of the steel sheet, and can contribute to improving the LME resistance. Therefore, the steel can contain B as necessary. While the lower limit of the B content is not particularly limited, in order to achieve the above effects, the B content is preferably made 0.0003% or more, more preferably 0.0005% or more, and even more preferably 0.0007% or more. However, if the B content exceeds 0.0100%, coarse precipitates will be formed, resulting in a reduction in ductility. Therefore, when the steel contains B, the B content is made 0.0090% or less. The B content is preferably made 0.0080% or less, more preferably 0.0070% or less, even more preferably 0.0050% or less, and most preferably 0.0030% or less.

### Cr: 1.00% or less

Cr has the effect of improving the balance between strength and ductility. Therefore, the steel can contain Cr as necessary. While the lower limit of the Cr content is not particularly limited, in order to achieve the above effect, the Cr content is preferably made 0.01% or more, more preferably 0.05% or more, and even more preferably 0.07% or more. However, if the steel contains Cr in an amount in excess of 1.00%, the area fraction of fresh martensite will be too high, resulting in a reduction in the dimensional accuracy and the ductility of the steel sheet during forming. Therefore, when the steel contains Cr, the Cr content is made 1.00% or less. The Cr content is preferably made 0.80% or less, more preferably 0.60% or less, even more preferably 0.50% or less, and most preferably 0.30% or less.

### Mo: 1.00% or less

Mo has the effect of improving the balance between strength and ductility. Therefore, the steel can contain Mo as necessary. While the lower limit of the Mo content is not particularly limited, in order to achieve the above effect, the Mo content is preferably made 0.01% or more, more preferably 0.05% or more, and even more preferably 0.07% or more. However, if the steel contains Mo in an amount in excess of 1.00%, the area fraction of fresh martensite will be too high, resulting in a reduction in the dimensional accuracy and the ductility of the steel sheet during forming. Therefore, when the steel contains Mo, the Mo content is made 1.00% or less. The Mo content is preferably made 0.80% or less, more preferably 0.50% or less, even more preferably 0.30% or less, and most preferably 0.20% or less.

### Co: 1.00% or less

Co is an element which is effective in improving the hardenability of the steel, and thus in strengthening the steel. Therefore, the steel can contain Co as necessary. While the lower limit of the Co content is not particularly limited, in order to achieve the above effect, the Co content is preferably made 0.01% or more, more preferably 0.05% or more, and even more preferably 0.07% or more. However, if the steel contains Co in an amount in excess of 1.00%, the area fraction of fresh martensite will be too high, resulting in a reduction in the dimensional accuracy and the ductility of the steel sheet during forming. Therefore, when the steel contains Co, the Co content is made 1.00% or less. The Co content is preferably made 0.80% or less, more preferably 0.60% or less, even more preferably 0.30% or less, and most preferably 0.20% or less.

### Ni: 1.00% or less

Ni increases the strength of the steel through solid solution strengthening. Therefore, the steel can contain Ni as necessary. While the lower limit of the Ni content is not particularly limited, in order to achieve the above effect, the Ni content is preferably made 0.01% or more, more preferably 0.05% or more, and even more preferably 0.07% or more. However, if the steel contains Ni in an amount in excess of 1.00%, the area fraction of fresh martensite will be too high, resulting in a reduction in the dimensional accuracy and the ductility of the steel sheet during forming. Therefore, when the steel contains Ni, the Ni content is made 1.00% or less. The Ni content is preferably made 0.80% or less, more preferably 0.60% or less, even more preferably 0.30% or less, and most preferably 0.20% or less.

### Cu: 1.00% or less

Cu is an element which is effective in strengthening the steel. Therefore, the steel can contain Cu as necessary. While the lower limit of the Cu content is not particularly limited, in order to achieve the above effect, the Cu content is preferably made 0.01% or more, more preferably 0.05% or more, and even more preferably 0.07% or more. However, if the steel contains Cu in an amount in excess of 1.00%, the area fractions of tempered martensite, bainite, and fresh martensite will be too high, resulting in a reduction in the dimensional accuracy and the ductility of the steel sheet during forming. Therefore, when the steel contains Cu, the Cu content is made 1.00% or less. The Cu content is preferably made 0.80% or less, more preferably 0.60% or less, even more preferably 0.30% or less, and most preferably 0.20% or less.

### Sn: 0.200% or less, Sb: 0.200% or less

Sn and Sb suppress decarburization in a surface region having a thickness of about a few tens of µm, caused by nitridation or oxidation of the surface of the steel sheet, thereby preventing a reduction in the area fraction of tempered martensite in the steel sheet surface. In addition to this effect, Sn and Sb have the effect of ensuring the strength and the material stability. Therefore, the steel can contain these elements as necessary. While the lower limit of the content of each element is not particularly limited, in order to achieve the above effects, the content of each element is preferably made 0.001% or more, more preferably 0.003% or more, and even more preferably 0.005% or more. However, if the content of each element exceeds 0.200%, the ductility of the steel sheet may be reduced due to embrittlement of the steel sheet. Therefore, when the steel contains Sn and Sb, the content of each element is made 0.200% or less. The content of each element is preferably 0.100% or less, more preferably 0.070% or less, even more preferably 0.050% or less, and most preferably 0.030% or less.

### Ca: 0.0100% or less, Mg: 0.0100% or less, REM: 0.0100% or less

The inclusion of Ca, Mg and REM in the steel, each in an amount of 0.0100% or less, causes no increase in the amount of coarse precipitates and inclusions and has no effect on the precipitation of Nb, and thus does not deteriorate the LME resistance. Therefore, when the steel contains Ca, Mg and REM, the content of each element is made 0.0100% or less. The content of each element is preferably made 0.0050% or less, more preferably 0.0040% or less, even more preferably 0.0035% or less, and most preferably 0.0030% or less. While the lower limit of the content of each element is not particularly specified, in view of the fact that each element makes the shape of a nitride or sulfide spherical and improves the limiting deformability of the steel sheet, the content of each of Ca, Mg and REM is preferably made 0.0001% or more, more preferably 0.0005% or more, even more preferably 0.0007% or more, and most preferably 0.0010% or more.

### Zr: 0.100% or less, Te: 0.100% or less

The inclusion of Zr and Te in the steel, each in an amount of 0.100% or less, causes no increase in the amount of coarse precipitates and inclusions and has no effect on the precipitation of Nb, and thus does not deteriorate the LME resistance. Therefore, when the steel contains Zr and Te, the content of each element is made 0.100% or less. The content of each element is preferably made 0.080% or less, more preferably 0.070% or less, even more preferably 0.060% or less, and most preferably 0.050% or less. While the lower limit of the content of each element is not particularly specified, in view of the fact that each element makes the shape of a nitride or sulfide spherical and improves the limiting deformability of the steel sheet, the content of each of Zr and Te is preferably made 0.001% or more, more preferably 0.010% or more, and even more preferably 0.020% or more.

### Hf: 0.10% or less

The inclusion of Hf in the steel in an amount of 0.10% or less causes no increase in the amount of coarse precipitates and inclusions and has no effect on the precipitation of Nb, and thus does not deteriorate the LME resistance. Therefore, when the steel contains Hf, the Hf content is made 0.10% or less. The Hf content is preferably made 0.080% or less, more preferably 0.070% or less, even more preferably 0.060% or less, and most preferably 0.050% or less. While the lower limit of the Hf content is not particularly specified, in view of the fact that Hf makes the shape of a nitride or sulfide spherical and improves the limiting deformability of the steel sheet, the Hf content is preferably made 0.003% or more, more preferably 0.010% or more, even more preferably 0.020% or more, and still more preferably 0.030% or more when the steel contains Hf.

### Bi: 0.200% or less

The inclusion of Bi in the steel in an amount of 0.200% or less causes no increase in the amount of coarse precipitates and inclusions and has no effect on the precipitation of Nb, and thus does not deteriorate the LME resistance. Therefore, when the steel contains Bi, the Bi content is made 0.200% or less. The Bi content is preferably made 0.100% or less, more preferably 0.050% or less, even more preferably 0.030% or less, and most preferably 0.020% or less. While the lower limit of the Bi content is not particularly specified, in view of the fact that Bi reduces segregation, the Bi content is preferably made 0.001% or more, more preferably 0.005% or more, and even more preferably 0.010% or more.

When the content of any of the above-described components V, Ta, W, B, Cr, Mo, Ni, Co, Cu, Sn, Sb, Ca, Mg, REM, Zr, Te, Hf and Bi is less than the preferred lower limit, the component does not impair the effects of the present invention and is regarded as an incidental impurity.

(2) A description will now be given of the microstructure.

### Area Fraction of Tempered Martensite and Bainite: not less than 40% and not more than 85%

Tempered martensite and bainite contribute to the strength of the steel sheet. In particular, to make the microstructure of the steel sheet composed mainly of tempered martensite and bainite is effective in maintaining a high strength. In order to fully achieve such an effect, the total area fraction of bainite and tempered martensite needs to be 40% or more. The total area fraction is preferably 42% or more, more preferably 45% or more, even more preferably 47% or more, and most preferably 50% or more. On the other hand, if the sum of the area fraction of bainite and the area fraction of tempered martensite exceeds 85%, the steel microstructure is occupied by hard phases including tempered martensite, bainite, and fresh martensite. In addition, such hard phases restrain retained austenite, and therefore the TRIP effect is not effectively exerted and the ductility is poor. Thus, it is difficult to achieve good formability. Therefore, the total area fraction of bainite and tempered martensite needs to be 85% or less. The total area fraction is preferably 83% or less, more preferably 82% or less, even more preferably 81% or less, and most preferably 80% or less.

### Area Fraction of Fresh Martensite: not less than 0% and not more than 25%

Fresh martensite is a very hard phase, and therefore increases the strength of the steel. Fresh martensite is not necessarily required if the strength of the steel sheet is secured; however, the inclusion of fresh martensite in the steel sheet microstructure can further increase the strength of the steel sheet, achieving further strengthening. Therefore, the area fraction of fresh martensite needs to be 0% or more. The area fraction is preferably 2% or more, more preferably 3% or more, even more preferably 4% or more, and most preferably 5% or more. On the other hand, fresh martensite reduces the ductility of the steel, making it difficult to achieve good formability. Therefore, the area fraction of fresh martensite needs to be 25% or less. The area fraction is preferably 23% or less, more preferably 22% or less, even more preferably 21% or less, and most preferably 20% or less.

### Area Fraction of Retained Austenite: not less than 5% and not more than 20%

Retained austenite transforms into martensite by the TRIP effect during processing. This increases the strength of the steel and, at the same time, enhances the strain dispersibility, thereby improving the ductility. In order to ensure good formability, the area fraction of retained austenite needs to be 5% or more. The area fraction is preferably 7% or more, more preferably 8% or more, even more preferably 9% or more, and most preferably 10% or more. On the other hand, if the area fraction of retained austenite exceeds 20%, elements concentrated in the retained austenite, especially Si, will diffuse during welding, causing a decrease in the melting point of zinc. This may facilitate the penetration of zinc into the steel sheet during welding, resulting in a deterioration of the LME resistance of the steel sheet. Therefore, in order to ensure sufficient ductility while preventing deterioration of the LME resistance, the area fraction of retained austenite needs to be 20% or less. The area fraction is preferably 18% or less, more preferably 17% or less, even more preferably 16% or less, and most preferably 15% or less.

In the present invention, the inclusion of a remaining microstructure, such as ferrite or pearlite, in the steel does not impair the effects of the present invention. When there is a remaining microstructure, it may include at least one of ferrite and pearlite, i.e., the area fraction of at least one of ferrite and pearlite may be 0% or more. The area fraction of the remaining microstructure is preferably 20% or less, more preferably 18% or less, even more preferably 15% or less, and most preferably 13% or less.

The relationship between the amount of dissolved Nb in the steel sheet (Nbₛₒₗ), the amount of Nb in Nb precipitates having a particle size of less than 20 nm (Nbₚᵣₑ), and the total amount of Nb contained in the steel sheet (Nb) satisfies the following Formula 1: $\left({Nb}_{sol}/Nb\right) + \left({Nb}_{pre}/Nb\right) \geq 0.40$ where Nbₛₒₗ represents the amount (mass %) of dissolved Nb, and Nbₚᵣₑ represents the amount (mass %) of Nb in Nb precipitates having a particle size of less than 20 nm.

To determine the relationship between the amount of dissolved Nb in the steel sheet (Nbₛₒₗ, unit: mass %), the amount of Nb in Nb precipitates having a particle size of less than 20 nm (Nbₚᵣₑ, unit: mass %), and the total amount of Nb contained in the steel sheet (Nb, unit: mass %) is one of the important factors of the present invention. In the present invention, Nb in the steel sheet is brought to a dissolved state, or to a state which can be converted into a dissolved state during welding, thereby preventing non-self-derived LME and improving the LME resistance. The present inventors, through experiments conducted using various steel sheets with varying states of Nb present therein, have found that the LME resistance is improved when Formula 1 is satisfied.

The mechanism by which Nb in the steel being in a dissolved state during welding improves the LME resistance is not clear, it is conceivable that when Nb exists in a dissolved state, it prevents the penetration of zinc into the steel sheet, which is the direct cause of LME cracking. Formula 1 thus needs to be satisfied. "(Nbₛₒₗ/Nb) + (Nbₚᵣₑ/Nb)" is preferably 0.41 or more, more preferably 0.42 or more. While the upper limit is not particularly limited, "(Nbₛₒₗ/Nb) + (Nbₚᵣₑ/Nb)" is preferably 0.95 or less, more preferably 0.90 or less. The lower limit of the particle size of the Nb precipitates is not particularly limited; for example, the Nb precipitates may have a particle size of 0.1 nm or more.

### Amount of Diffusible Hydrogen in Steel: 0.50 mass ppm or less

In order to ensure good ductility and thus good formability, the amount of diffusible hydrogen in the steel is made 0.50 mass ppm or less. The amount of diffusible hydrogen is preferably made 0.30 mass ppm or less, more preferably 0.25 mass ppm or less, even more preferably 0.20 mass ppm or less, and most preferably 0.15 mass ppm or less. While the lower limit of the amount of diffusible hydrogen in the steel is not particularly specified, in view of the restrictions of production technology, the amount of diffusible hydrogen is preferably made 0.01 mass ppm or more, more preferably 0.02 mass ppm or more, even more preferably set to 0.03 mass ppm or more, and most preferably 0.05 mass ppm or more.

(3) A manufacturing method and manufacturing conditions will now be described.

### [Slab (Steel Material) Heating Step]

Steel Material Heating Conditions: heating for 1.0 hours or more at a temperature equal to or higher than Tₛₒₗ°C represented by Formula 2
Precipitates existing in the heating stage of the steel material will exist as coarse precipitates in the steel sheet finally obtained, which not only adversely affects the LME resistance, but does not contribute to the strength, and thus does not improve the TS × El balance. Therefore, coarse precipitates, which have been precipitated during casting, need to be re-dissolved as much as possible. If the steel material heating temperature is below Tₛₒₗ°C or the heating time is less than one hour, the dissolution of Nb will be insufficient, and Formula 1 will not be satisfied. This may result in poor LME resistance and in an increased risk of trouble during hot rolling due to an increase in rolling load. Also from the viewpoint of scaling off defects such as bubbles and segregations in the surface of the steel material, and reducing cracking and unevenness on the surface of the steel sheet, thereby achieving a smooth surface, the steel material heating temperature needs to be equal to or higher than Tₛₒₗ°C. Therefore, the steel material heating temperature is made equal to or higher than Tₛₒₗ°C represented by the following Formula 2. The steel material heating temperature is preferably equal to or higher than "Tₛₒₗ × 1.1"°C, more preferably equal to or higher than "Tₛₒₗ × 1.2"°C, even more preferably equal to or higher than "Tₛₒₗ × 1.3"°C, and most preferably equal to or higher than "Tₛₒₗ × 1.5"°C. The heating time at the temperature is made 1.0 hours or more. The heating time is preferably 1.1 hours or more, more preferably 1.2 hours or more, even more preferably 1.3 hours or more, and most preferably 1.5 hours or more. While the upper limit of the steel material heating temperature is not particularly specified, the use of a heating temperature exceeding 1500°C increases the amount of oxidation, resulting in an increased scale loss. Therefore, the steel material heating temperature is preferably made 1500°C or lower, more preferably 1450°C or lower, and even more preferably 1400°C or lower. ${T}_{sol} = 7900 / \left(3.42-\left(log\left(\left[Nb%\right]\left[C%\right]\right)\right)\right) - 273$

### [Hot Rolling Step]

### Finish Rolling Start Temperature in Hot Rolling: T_{FET}°C

The steel material after the heating is hot-rolled into a hot-rolled steel sheet. While the upper and lower limits of the start temperature of finish rolling in the hot rolling are not particularly specified, a finish rolling start temperature of less than "Tₛₒₗ°C - 100°C" will cause precipitation of Nb which has been dissolved during heating of the steel material, resulting in an increase in the particle size of precipitates. Accordingly, Formula 1 may not be satisfied, and thus the LME resistance may be poor. Therefore, the finish rolling start temperature is preferably made "Tₛₒₗ°C - 100°C" or higher, more preferably "Tₛₒₗ°C - 70°C" or higher, even more preferably "Tₛₒₗ°C - 50°C" or higher, and most preferably "Tₛₒₗ°C - 30°C" or higher. On the other hand, a finish rolling start temperature exceeding 1200°C may increase a scale loss during pre-heating of the slab, causing breakage of the sheet during hot rolling. Therefore, the finish rolling start temperature in hot rolling is preferably made 1200°C or lower, more preferably 1170°C or lower, even more preferably 1150°C or lower, and most preferably 1120°C or lower.

### Finish Rolling Delivery Temperature in Hot Rolling: T_{FDT}°C

The steel material after the heating is hot-rolled into a hot-rolled steel sheet. While the upper and lower limits of the delivery temperature in the finish rolling are not particularly specified, a finish rolling delivery temperature of less than 800°C will cause precipitation of Nb which has been dissolved during heating of the steel material, resulting in an increase in the amount of Nb precipitated. Further, such a delivery temperature increases a rolling load, and thus a rolling burden, which may impede a cold rolling process. Therefore, the finish rolling delivery temperature in hot rolling is preferably made 800°C or higher, more preferably 820°C or higher, even more preferably 840°C or higher, and most preferably 850°C or higher. If the finish temperature exceeds 1000°C, the amount of oxides (scale) produced tends to increase rapidly, resulting in roughening of the interface between the base steel and the oxides, and deterioration of the surface quality after pickling and cold rolling. In addition, crystal grains may become excessively coarse, causing surface roughening of the pressed product during processing. Therefore, the finish rolling delivery temperature is preferably made 1000°C or lower, more preferably 980°C or lower, even more preferably 970°C or lower, and most preferably 950°C or lower.

### Effective Time: t_{HR}

Effective time t_{HR} is herein defined as the time required from the start of finish rolling to the end of finish rolling. Since Nb contained in the steel sheet begins to precipitate and grow during finish rolling, the effective time t_{HR} is one of the parameters for controlling the form of Nb to improve the LME resistance. While the upper and lower limits of the effective time t_{HR} are not particularly specified, the effective time t_{HR} is preferably made 3 seconds or more, more preferably 4 seconds or more, even more preferably 5 seconds or more, and most preferably 7 seconds or more. The effective time t_{HR} is preferably made 15 seconds or less, more preferably 12 seconds or less, even more preferably 11 seconds or less, and most preferably 10 seconds or less.

### [Coiling Step]

### Residence Time from T_{FDT}°C to 650°C: t_{CT}

Residence time t_{CT} is herein defined as the time from the finish rolling delivery temperature to 650°C. Since the precipitation of Nb and the growth of precipitated Nb are likely to proceed during the period from the completion of finish rolling to the sheet temperature reaching 650°C, the residence time t_{CT} is one of the parameters for controlling the form of Nb to improve the LME resistance. While the upper and lower limits of the residence time t_{CT} are not particularly specified, the residence time t_{CT} is preferably made 5 seconds or more, more preferably 7 seconds or more, even more preferably 8 seconds or more, and most preferably 9 seconds or more. The residence time t_{CT} is made 20 seconds or less, more preferably 18 seconds or less, even more preferably 17 seconds or less, and most preferably 15 seconds or less.

### Coiling Temperature T_{CT}°C after Hot Rolling: 650°C or lower

If the coiling temperature after hot rolling is higher than 650°C, the precipitation of Nb and the growth of precipitated Nb may proceed excessively, so that Formula 1 may not be satisfied. This causes deterioration of the LME resistance and, in addition, causes the formation of an oxide film, which is difficult to remove by pickling, on the surface of the hot-rolled sheet, which may impair the surface appearance of the steel sheet after cold rolling. Therefore, the coiling temperature after hot rolling is made 650°C or lower. The coiling temperature is preferably 630°C or lower, more preferably 620°C or lower, even more preferably 610°C or lower, and most preferably 600°C or lower. While the lower limit of the coiling temperature is not particularly limited, if the coiling temperature is lower than 300°C, the strength of the hot-rolled sheet increases, which may cause an increase in the rolling burden in cold rolling and a defective sheet shape, resulting in a reduction in productivity. Therefore, the lower limit of the coiling temperature is preferably made 300°C or higher, more preferably 320°C or higher, even more preferably 350°C or higher, and most preferably 400°C or higher.

The resulting hot-rolled steel sheet (hot-rolled coil) may be subjected to intermediate heat treatment at a temperature below 650°C, as necessary, to prevent an increase in load in later cold rolling. The heat treatment is preferably performed at a temperature of 150°C or higher. The heat treatment may be carried out, for example, in a box annealing furnace at a soaking temperature of 500°C for a soaking time of 4 hours.

The resulting hot-rolled steel sheet (hot-rolled coil) may be subjected to a treatment, such as pickling, as necessary. Pickling of the hot-rolled coil may be performed by a common method. The hot-rolled coil may also be subjected to skin pass rolling to correct its shape and enhance its pickling properties.

After the hot rolling and/or the intermediate heat treatment and/or the pickling, the steel sheet may be subjected directly to the below-described annealing step (heat treatment), or may be subjected to cold rolling prior to the heat treatment. When cold rolling is performed, the cold rolling reduction is preferably made 25% or more, more preferably 30% or more, even more preferably 32% or more, and most preferably 35% or more. On the other hand, an excessive reduction causes a too-high rolling load, leading to an increase in the burden on a cold rolling mill. Therefore, the cold rolling reduction is preferably made 75% or less, more preferably 70% or less, even more preferably 67% or less, and most preferably 65% or less.

### [Annealing Step]

### Heating Time from 650°C to Soaking Temperature T_{AT}°C: t

The precipitation of Nb and the growth of precipitated Nb proceeds at a sheet temperature of 650°C or higher. Thus, the heating time t is one of the parameters for controlling the form of Nb to improve the LME resistance. While the upper and lower limits of the heating time t are not particularly specified, the heating time t is preferably made 300 seconds or more, more preferably 400 seconds or more, even more preferably 450 seconds or more, and most preferably 490 seconds or more. The heating time t is preferably made 700 seconds or less, more preferably 650 seconds or less, even more preferably 600 seconds or less, and most preferably 590 seconds or less.

### Soaking Temperature: T_{AT} not less than 750°C and not more than 950°C

When the steel sheet is held in a temperature range below 750°C, it is held in a two-phase region. In such a case, the total area fraction of tempered martensite and bainite in the final microstructure is less than 40%, and therefore a sufficient steel sheet strength cannot be ensured. Therefore, the soaking temperature T_{AT}°C is made 750°C or higher, preferably 770°C or higher, more preferably 800°C or higher, and even more preferably 840°C or higher. On the other hand, if the steel sheet is held in a temperature range above 950°C, the precipitation of Nb is promoted, and the growth of Nb precipitates proceeds excessively. Accordingly, Formula 1 will not be satisfied, leading to a reduction in the LME resistance. Therefore, the soaking temperature T_{AT}°C is made 950°C or lower, preferably 940°C or lower, more preferably 930°C or lower, and even more preferably 920°C or lower.

### Holding Time at Soaking Temperature T_{AT}°C: t_{AT}

Holding time t_{AT} at the soaking temperature T_{AT}°C is one of the control parameters for promoting austenitizing of the steel sheet during soaking and, since it is related to the precipitation of Nb and the growth of Nb precipitates, is also one of the parameters for controlling the LME resistance. While the upper and lower limits of the holding time t_{AT} are not particularly specified, the holding time t_{AT} is preferably made 15 seconds or more in order to sufficiently promote austenitizing. The holding time t_{AT} is more preferably made 30 seconds or more, even more preferably 50 seconds or more, and most preferably 100 seconds or more. On the other hand, from the viewpoint of making the particles of Nb precipitates finer to improve the LME resistance, the holding time t_{AT} is preferably made 1000 seconds or less, more preferably 500 seconds or less, even more preferably 400 seconds or less, and most preferably 350 seconds or less.

### Sum of Q_{HR}, Q_{CT} and Q_{AT}: 6000 or less

In order to suppress the precipitation of Nb and the growth of Nb precipitates during heating in the hot rolling step, the coiling step, and the annealing step, the following is an important requirement in the present invention for reasons which will be described below: Q_{HR} defined by the following Formula 3 in terms of the finish rolling start temperature T_{FET}°C, the finish rolling delivery temperature T_{FDT}°C, and the effective time t_{HR} from the start of finish rolling to the end of finish rolling, Q_{CT} defined by the following Formula 4 in terms of the residence time t_{CT} from T_{FDT}°C to 650°C and the coiling temperature T_{CT}°C in the coiling step, and Q_{AT} defined by the following Formula 5 in terms of the soaking temperature T_{AT}°C, the heating time t from 650°C to the soaking temperature T_{AT}°C, and the holding time t_{AT} at the soaking temperature T_{AT}°C in the annealing step, satisfy the following Formula 6, i.e., the sum of Q_{HR}, Q_{CT}, and Q_{AT} is 6000 or less. ${Q}_{HR} = 0.5 \left({T}_{FET}+{T}_{FDT}\right) \times {log}_{10} \left({t}_{HR}\right)$ ${Q}_{CT} = 0.5 \left({T}_{CT}+650\right) \times {log}_{10} \left({t}_{CT}\right)$ ${Q}_{AT} = 0.5 \left(650+{T}_{AT}\right) \times {log}_{10} \left(t\right) + {T}_{AT} \times {log}_{10} \left({t}_{AT}\right)$ ${Q}_{HR} + {Q}_{CT} + {Q}_{AT} \leq 6000$

That the sum of Q_{HR}, Q_{CT}, and Q_{AT} is 6000 or less is an important requirement in the present invention in order to suppress the precipitation and growth of Nb in the hot rolling step, the coiling step, and the heating step. As described above, Q_{HR}, Q_{CT}, and Q_{AT} are each defined by the temperatures at the start and end of each of the effective time t_{HR}, the residence time t_{CT}, the heating time t, and the holding time t_{AT}, during which heat of 650°C to Tₛₒₗ is applied.

If the sum of Q_{HR}, Q_{CT}, and Q_{AT} exceeds 6000, Nb will be precipitated excessively and the precipitates will grow excessively, and thus the amount of Nb that improves the LME resistance will decrease, resulting in poor LME resistance. Therefore, the sum of Q_{HR}, Q_{CT}, and Q_{AT} is made 6000 or less, preferably 5990 or less, more preferably 5980 or less, even more preferably 5970 or less, and most preferably 5950 or less. While the lower limit of the sum of Q_{HR}, Q_{CT}, and Q_{AT} is not particularly specified, in view of the feasible range in actual operations, the sum is preferably made 3500 or more, more preferably 3600 or more, even more preferably 3700 or more, most preferably 3800 or more, and particularly preferably 3900 or more.

### Q_{AT} Value of 4700 or Less (Preferred Condition)

From the viewpoint of taking account of the total heat applied during heating in the hot rolling step, the coiling step, and the annealing step to suppress excessive precipitation and growth of Nb, its evaluation is performed based on the sum of Q_{HR}, Q_{CT}, and Q_{AT}. Therefore, the upper and lower limits of each parameter are not particularly specified. However, from the viewpoint of suppressing excessive growth of Nb during heating in the annealing step, which directly leads to the final microstructure of the steel sheet, Q_{AT} is preferably made 4700 or less, more preferably 4650 or less, even more preferably 4630 or less, and most preferably 4600 or less. From the viewpoint of more precisely controlling the austenite fraction during annealing in order to increase the strength of the steel, Q_{AT} is preferably made 3500 or more, more preferably 3800 or more, even more preferably 4100 or more, and most preferably 4120 or more.

Likewise for the hot rolling step and the coiling step, from the viewpoint of suppressing excessive growth of Nb, Q_{HR} is preferably made 1200 or less, more preferably 1170 or less, and even more preferably 1150 or less. Q_{CT} is preferably made 850 or less, more preferably 840 or less, and even more preferably 835 or less. On the other hand, while no particular limitation is placed especially on the lower limit of Q_{HR}, Q_{HR} is preferably made 250 or more, more preferably 600 or more, and even more preferably 700 or more. Q_{CT} is preferably made 150 or more, more preferably 170 or more, and even more preferably 180 or more.

In the annealing step, after the steel sheet is held at the soaking temperature T_{AT} for the holding time t_{AT}, the steel sheet may be simply cooled, may be cooled to an arbitrary holding temperature and held at the temperature, and then cooled again, or may be cooled to an arbitrary cooling stop temperature, then reheated to a holding temperature and held at the temperature, and then cooled again.

After the annealing step, the steel sheet may be reheated. When martensite is formed in the steel sheet and then tempered, C is concentrated in untransformed austenite. This enhances the stability of austenite and increases the area fraction of retained austenite contained in the steel sheet after cooling, making it possible to further enhance the ductility. When the steel sheet is reheated for such reasons, it is preferred to cool the steel sheet to a cooling stop temperature of not less than 100°C and not more than 350°C, reheat the steel sheet to a holding temperature of not less than 200°C and not more than 450°C, hold the steel sheet at the temperature, and then cool the steel sheet to room temperature. The reheating temperature is preferably made 200°C or higher, more preferably 210°C or higher, even more preferably 230°C or higher, and most preferably 250°C or higher. The reheating temperature is preferably made 450°C or lower, more preferably 430°C or lower, even more preferably 410°C or lower, and most preferably 400°C or lower.

When reheating of the steel sheet is not performed, it is preferred to hold the steel sheet at a holding temperature of not less than 200°C and not more than 450°C for 10 seconds or more, and then cool the steel sheet to room temperature. The steel sheet is more preferably held at a holding temperature of not less than 200°C and not more than 450°C for 20 seconds or more, even more preferably for 25 seconds or more. While the upper limit of the holding time is not particularly limited, the holding time is preferably made 500 seconds or less, more preferably 400 seconds or less.

### Coating Treatment

When the steel sheet is subjected to hot-dip galvanizing, for example, the steel sheet which has undergone the above-described annealing treatment is immersed in a galvanizing bath at 440°C to 500°C to perform hot-dip galvanizing of the steel sheet, followed by gas wiping or the like to adjust the coating weight. The temperature of the galvanizing bath is preferably made 440°C or higher, more preferably 450°C or higher, and even more preferably 455°C or higher. The temperature of the galvanizing bath is preferably made 500°C or lower, more preferably 490°C or lower, and even more preferably 485°C or lower.

While there is no particular restriction placed on the coating conditions, the coating weight (per one surface) is preferably 20 g/m² or more from the viewpoint of corrosion resistance and control of the coating weight. The coating weight is more preferably 25 g/m² or more, even more preferably 30 g/m² or more, and most preferably 32 g/m² or more. From the viewpoint of adhesion, the coating weight is preferably 120 g/m² or less, more preferably 100 g/m² or less, even more preferably 70 g/m² or less, and most preferably 65 g/m² or less.

The hot-dip galvanizing is preferably performed using a galvanizing bath containing 0.08% to 0.30% of Al. Thus, the amount of Al in the hot-dip galvanizing is preferably made 0.08% or more, more preferably 0.09% or more, even more preferably 0.10% or more, and most preferably 0.12% or more. The amount of Al in the hot-dip galvanizing is preferably made 0.30% or less, more preferably 0.25% or less, even more preferably 0.22% or less, and most preferably 0.20% or less. If elements other than Al, Mg, and Si, such as Pb, Sb, Fe, Mg, Mn, Ni, Ca, Ti, V, Cr, Co, and Sn are mixed into the galvanizing bath, such elements will not significantly affect the effects of the present invention.

When an alloying treatment is performed on a galvanized coating, the treatment is performed in a temperature range of 450°C to 600°C. If the alloying treatment is performed at a temperature exceeding 600°C, untransformed austenite will be transformed into pearlite, and the area fraction of retained austenite will be less than 5%, which may result in a reduction in ductility. Therefore, when an alloying treatment of a galvanized coating is performed, the alloying treatment is preferably performed in a temperature range of not less than 450°C, more preferably not less than 460°C, even more preferably not less than 465°C, and most preferable not less than 470°C. Further, when an alloying treatment of a galvanized coating is performed, the alloying treatment is preferably performed in a temperature range of not more than 600°C, more preferably not more than 570°C, even more preferably not more than 550°C, and most preferably not more than 530°C. The alloyed coating layer of the hot-dip galvanized steel sheet preferably has an Fe concentration of 8% to 17%. Thus, the Fe concentration of the alloyed coating layer of the hot-dip galvanized steel sheet is preferably 8% or more, more preferably 9% or more, and even more preferably 10% or more. The Fe concentration of the alloyed coating layer of the hot-dip galvanized steel sheet is preferably 17% or less, more preferably 16% or less, and even more preferably 15% or less. The alloyed coating layer is thus formed by performing the alloying treatment on the hot-dip galvanized steel sheet.

### EXAMPLES

Molten steels having the chemical compositions shown in Tables 1-1 and 1-2, with the balance being Fe and incidental impurities, were produced in a converter. Each molten steel was continuously cast into a slab. The slab was subjected to a heating step, a hot rolling step, a coiling step, and an annealing (heating) step under the conditions shown in Tables 2-1 and 2-2. When reheating of the steel sheet was performed, the steel sheet after annealing was cooled to a cooling stop temperature of 100°C to 350°C, reheated to a holding temperature of 200°C to 450°C, held at the holding temperature, and then cooled to room temperature. When reheating of the steel sheet was not performed, the steel sheet after annealing was held at a holding temperature of 200°C to 450°C for 10 seconds or more, and then cooled to room temperature. In either case, the cooled steel sheet was cold-rolled at a rolling reduction of 50% to obtain a high-strength cold-rolled steel sheet (CR). Some steel sheets after the coiling step were subjected to the heating step, but were not subjected to cold rolling, to obtain hot-rolled steel sheets (HR). Some steel sheets were subjected to hot-dip galvanizing to obtain hot-dip galvanized steel sheets (GI) and galvannealed steel sheets (GA). A galvanizing bath containing 0.19 mass % Al was used for the hot-dip galvanized steel sheets (GI), and a galvanizing bath containing 0.14 mass % Al was used for the galvannealed steel sheets (GA). The temperature of each bath was 465°C. The coating weight was 45 g/m² per one surface (double-sided coating). For the galvannealed steel sheets (GA), the Fe concentration in the coating layer was adjusted to be within the range of 9 mass % to 12 mass %.

Each of the resulting steel sheets was examined for its cross-sectional microstructure, tensile properties, and LME resistance, the results of which are shown in Tables 3-1 and 3-2.

**[Table 2-1]**

| | | Heating step | | | Hot rolling step | | | | Coiling step | | | Annealing step | | | | | | |
|---|---|---|---|---|---|---|---|---|---|---|---|---|---|---|---|---|---|---|
| Steel sheet sample No. | Steel symbol | Tₛₒₗ (°C) | Heating temp. T (°C) | Heating time (hour) | Finish rolling start temp. T_{FET} (°C) | Finish rolling delivery temp. T_{FDT} (°C) | Effective time t_{HR} (sec) | Q_{HR} (°C·sec) | Residence time t_{CT} (sec) | Coiling temp. T_{CT} (°C) | Q_{CT} (°C·sec) | Heating time t (sec) | Soaking temp. T_{AT} (°C) | Holding time t_{AT} (sec) | Q_{AT} (°C·sec) | Q_{HR} + Q_{CT} + Q_{AT} (°C·sec) | Re- heated? | State of steel sheet |
| 1 | A | 899 | 1270 | 1.8 | 1080 | 920 | 6 | 778 | 14 | 560 | 693 | 580 | 880 | 280 | 4268 | 5739 | yes | CR |
| 2 | A | 899 | 1270 | 1.8 | 1080 | 920 | 7 | 845 | 6 | 510 | 451 | 480 | 870 | 260 | 4139 | 5435 | no | CR |
| 3 | B | 1038 | 1260 | 1.3 | 1110 | 970 | 7 | 879 | 12 | 574 | 660 | 570 | 920 | 260 | 4385 | 5924 | yes | CR |
| 4 | B | 1038 | 1260 | 1.3 | 1060 | 970 | 4 | 611 | 11 | 590 | 646 | 560 | 880 | 240 | 4197 | 5454 | no | CR |
| 5 | C | 1072 | 1290 | 1.1 | 1060 | 940 | 6 | 778 | 11 | 590 | 646 | 570 | 850 | 280 | 4147 | 5571 | yes | CR |
| 6 | C | 1072 | 1290 | 1.1 | 1100 | 940 | 8 | 921 | 15 | 500 | 676 | 550 | 860 | 230 | 4100 | 5697 | no | CR |
| 7 | C | 1072 | 1290 | 1.1 | 1070 | 940 | 6 | 782 | 11 | 490 | 594 | 540 | 920 | 250 | 4351 | 5727 | yes | GA |
| 8 | C | 1072 | 1290 | 1.1 | 1110 | 940 | 6 | 798 | 9 | 540 | 568 | 580 | 920 | 290 | 4435 | 5801 | yes | GI |
| 9 | C | 1072 | 1250 | 1.4 | 1110 | 950 | 6 | 801 | 8 | 550 | 542 | 580 | 900 | 290 | 4358 | 5701 | yes | HR |
| 10 | D | 1101 | 1280 | 1.3 | 1110 | 900 | 7 | 849 | 6 | 570 | 475 | 500 | 890 | 290 | 4270 | 5594 | yes | CR |
| 11 | D | 1101 | 1280 | 1.3 | 1110 | 900 | 7 | 849 | 9 | 510 | 553 | 540 | 860 | 280 | 4168 | 5570 | no | CR |
| 12 | D | 1101 | 1070 | 1.3 | 1040 | 900 | 7 | 820 | 13 | 610 | 702 | 550 | 880 | 300 | 4276 | 5798 | yes | CR |
| 13 | D | 1101 | 1280 | 0.4 | 1120 | 900 | 7 | 854 | 12 | 540 | 642 | 580 | 860 | 280 | 4191 | 5687 | yes | CR |
| 14 | D | 1101 | 1280 | 1.3 | 1060 | 900 | 6 | 763 | 9 | 700 | 644 | 440 | 900 | 240 | 4191 | 5598 | yes | CR |
| 15 | D | 1101 | 1280 | 1.3 | 1060 | 900 | 4 | 590 | 13 | 560 | 674 | 550 | 980 | 250 | 4583 | 5847 | yes | CR |
| 16 | D | 1101 | 1280 | 1.3 | 1090 | 900 | 5 | 695 | 8 | 560 | 546 | 500 | 720 | 240 | 3563 | 4804 | yes | CR |
| 17 | D | 1101 | 1280 | 1.3 | 1160 | 960 | 14 | 1215 | 6 | 570 | 475 | 560 | 890 | 300 | 4321 | 6011 | yes | CR |
| 18 | D | 1101 | 1280 | 1.3 | 1160 | 960 | 7 | 896 | 21 | 640 | 853 | 560 | 890 | 300 | 4321 | 6070 | yes | CR |
| 19 | D | 1101 | 1280 | 1.3 | 1160 | 960 | 7 | 896 | 6 | 570 | 475 | 560 | 940 | 500 | 4722 | 6093 | yes | CR |
| 20 | D | 1101 | 1280 | 1.3 | 1160 | 960 | 7 | 896 | 15 | 500 | 676 | 550 | 950 | 230 | 4436 | 6008 | yes | CR |
| 21 | D | 1101 | 1280 | 1.3 | 1110 | 870 | 2 | 298 | 9 | 530 | 563 | 510 | 910 | 240 | 4278 | 5139 | no | CR |
| 22 | E | 1205 | 1300 | 1.8 | 1150 | 950 | 6 | 817 | 10 | 520 | 585 | 520 | 900 | 300 | 4334 | 5736 | yes | CR |
| 23 | F | 1015 | 1240 | 1.5 | 1120 | 900 | 5 | 706 | 14 | 600 | 716 | 520 | 870 | 260 | 4165 | 5587 | yes | CR |
| 24 | G | 1205 | 1300 | 1.3 | 1120 | 880 | 12 | 1079 | 8 | 610 | 569 | 490 | 920 | 250 | 4318 | 5966 | yes | CR |
| 25 | H | 1107 | 1140 | 1.4 | 1080 | 890 | 6 | 766 | 8 | 510 | 524 | 490 | 850 | 280 | 4098 | 5388 | yes | CR |
| 26 | I | 1013 | 1230 | 1.5 | 1060 | 970 | 7 | 858 | 7 | 510 | 490 | 520 | 890 | 120 | 3942 | 5290 | yes | CR |
| 27 | J | 996 | 1220 | 1.0 | 1060 | 980 | 6 | 794 | 8 | 610 | 569 | 510 | 920 | 260 | 4347 | 5710 | yes | CR |
| 28 | K | 1015 | 1470 | 1.9 | 1190 | 800 | 5 | 695 | 13 | 560 | 674 | 550 | 930 | 250 | 4395 | 5764 | yes | CR |
| 29 | L | 1140 | 1280 | 1.8 | 1140 | 860 | 5 | 699 | 8 | 580 | 555 | 480 | 880 | 240 | 4146 | 5400 | yes | CR |
| 30 | M | 1146 | 1250 | 1.5 | 1120 | 930 | 7 | 866 | 10 | 650 | 650 | 550 | 850 | 270 | 4122 | 5638 | yes | CR |
| 31 | N | 1067 | 1310 | 1.7 | 1130 | 880 | 6 | 782 | 9 | 550 | 573 | 470 | 870 | 260 | 4132 | 5487 | yes | CR |
| 32 | O | 785 | 1260 | 1.1 | 1110 | 950 | 5 | 720 | 9 | 500 | 549 | 440 | 880 | 240 | 4117 | 5386 | yes | CR |
| 33 | P | 1192 | 1300 | 1.4 | 1070 | 910 | 7 | 837 | 15 | 550 | 706 | 460 | 860 | 300 | 4141 | 5684 | yes | CR |
| 34 | Q | 1096 | 1280 | 1.1 | 1120 | 900 | 6 | 786 | 13 | 560 | 674 | 560 | 860 | 120 | 3863 | 5323 | yes | CR |
| 35 | R | 1092 | 1280 | 1.3 | 1070 | 940 | 7 | 849 | 12 | 500 | 621 | 580 | 920 | 250 | 4375 | 5845 | yes | CR |
| 36 | S | 1045 | 1270 | 1.2 | 1080 | 960 | 8 | 921 | 10 | 580 | 615 | 480 | 870 | 200 | 4040 | 5576 | yes | CR |
| 37 | T | 1076 | 1330 | 1.9 | 1080 | 910 | 7 | 841 | 6 | 580 | 479 | 520 | 940 | 260 | 4429 | 5749 | yes | CR |
| 38 | U | 1061 | 1290 | 1.4 | 1070 | 900 | 9 | 940 | 5 | 540 | 416 | 560 | 940 | 300 | 4513 | 5869 | yes | CR |
| 39 | V | 1018 | 1240 | 1.0 | 1100 | 900 | 4 | 602 | 10 | 520 | 585 | 520 | 900 | 300 | 4334 | 5521 | yes | CR |
| 40 | W | 1049 | 1230 | 1.0 | 1090 | 920 | 8 | 908 | 9 | 580 | 587 | 560 | 870 | 260 | 4190 | 5685 | yes | CR |
| 41 | X | 1170 | 1230 | 1.0 | 1120 | 900 | 8 | 912 | 10 | 500 | 575 | 570 | 930 | 250 | 4407 | 5894 | yes | CR |
| 42 | Y | - | 1280 | 1.1 | 1090 | 870 | 9 | 935 | 12 | 500 | 621 | 500 | 950 | 230 | 4403 | 5959 | yes | CR |
| 43 | Z | 1653 | 1680 | 1.7 | 1090 | 950 | 5 | 713 | 10 | 510 | 580 | 460 | 920 | 280 | 4342 | 5635 | yes | CR |

| | | | | | | | | | | | | | | | | | | |
|---|---|---|---|---|---|---|---|---|---|---|---|---|---|---|---|---|---|---|
| * HR: hot-rolled steel sheet (no coating), CR: cold-rolled steel sheet (no coating), GI: hot-dip galvanized steel sheet (no alloying of galvanized coating), GA: galvannealed steel sheet The underlines indicate that the values are outside the scope of the present invention. | | | | | | | | | | | | | | | | | | |

**[Table 2-2]**

| | | Heating step | | | Hot rolling step | | | | Coiling step | | | Annealing step | | | | | | |
|---|---|---|---|---|---|---|---|---|---|---|---|---|---|---|---|---|---|---|
| Steel sheet sample No. | Steel symbol | Tsol (°C) | Heating temp. T (°C) | Heating time (hour) | Finish rolling start temp. T_{FET} (°C) | Finish rolling delivery temp. TFDT (°C) | Effective time t_{HR} (sec) | Q_{HR} (°C·sec) | Residence time t_{CT} (sec) | Coiling temp. T_{CT} (°C) | Q_{CT} (°C·sec) | Heating time t (sec) | Soaking temp. T_{AT} (°C) | Holding time t_{AT} (sec) | Q_{AT} (°C·sec) | Q_{HR} + Q_{CT} + Q_{AT} (°C·sec) | Reheated? | State of steel sheet |
| 44 | AA | 1042 | 1320 | 1.4 | 1060 | 890 | 7 | 824 | 9 | 510 | 553 | 540 | 860 | 280 | 4168 | 5545 | yes | CR |
| 45 | AB | 1072 | 1310 | 2.0 | 1120 | 890 | 5 | 702 | 12 | 540 | 642 | 490 | 860 | 280 | 4136 | 5480 | yes | CR |
| 46 | AC | 1126 | 1330 | 2.0 | 1070 | 920 | 10 | 995 | 14 | 640 | 739 | 520 | 860 | 300 | 4181 | 5915 | yes | CR |
| 47 | AD | 1078 | 1290 | 1.6 | 1120 | 950 | 9 | 988 | 15 | 580 | 723 | 490 | 900 | 240 | 4227 | 5938 | yes | CR |
| 48 | AE | 1142 | 1270 | 1.1 | 1100 | 880 | 8 | 894 | 11 | 590 | 646 | 560 | 880 | 240 | 4197 | 5737 | yes | CR |
| 49 | AF | 1108 | 1310 | 1.3 | 1060 | 860 | 6 | 747 | 15 | 580 | 723 | 430 | 880 | 300 | 4194 | 5664 | yes | CR |
| 50 | AG | 1012 | 1280 | 1.1 | 1120 | 960 | 8 | 939 | 14 | 600 | 716 | 520 | 870 | 260 | 4165 | 5820 | yes | CR |
| 51 | AH | 1097 | 1230 | 1.0 | 1090 | 910 | 4 | 602 | 13 | 510 | 646 | 580 | 910 | 270 | 4368 | 5616 | yes | CR |
| 52 | AI | 1095 | 1310 | 1.7 | 1080 | 890 | 9 | 940 | 8 | 540 | 537 | 500 | 910 | 300 | 4359 | 5836 | yes | CR |
| 53 | AJ | 1083 | 1260 | 1.9 | 1050 | 970 | 6 | 786 | 16 | 500 | 692 | 500 | 920 | 240 | 4308 | 5786 | yes | CR |
| 54 | AK | 1104 | 1280 | 1.1 | 1070 | 960 | 6 | 790 | 10 | 580 | 615 | 580 | 890 | 320 | 4357 | 5762 | yes | CR |
| 55 | AL | 1128 | 1310 | 1.3 | 1080 | 860 | 7 | 820 | 14 | 650 | 745 | 440 | 910 | 240 | 4228 | 5793 | yes | CR |
| 56 | AM | 1065 | 1220 | 2.0 | 1120 | 950 | 9 | 988 | 9 | 530 | 563 | 510 | 910 | 240 | 4278 | 5829 | yes | CR |
| 57 | AN | 1079 | 1310 | 1.7 | 1050 | 950 | 6 | 778 | 11 | 590 | 646 | 570 | 850 | 280 | 4147 | 5571 | yes | CR |
| 58 | AO | 1135 | 1260 | 1.5 | 1110 | 970 | 7 | 879 | 12 | 540 | 642 | 580 | 920 | 300 | 4448 | 5969 | yes | CR |
| 59 | AP | 1125 | 1280 | 1.6 | 1060 | 860 | 6 | 747 | 13 | 610 | 702 | 550 | 880 | 300 | 4276 | 5725 | yes | CR |
| 60 | AQ | 1121 | 1240 | 1.3 | 1050 | 890 | 9 | 926 | 19 | 580 | 786 | 620 | 860 | 300 | 4239 | 5951 | yes | CR |
| 61 | AR | 1134 | 1250 | 1.1 | 1090 | 890 | 5 | 692 | 19 | 580 | 786 | 620 | 860 | 300 | 4239 | 5717 | yes | CR |
| 62 | AS | 1120 | 1210 | 1.4 | 1120 | 950 | 6 | 805 | 13 | 510 | 646 | 590 | 880 | 300 | 4300 | 5751 | yes | CR |
| 63 | AT | 1101 | 1230 | 1.3 | 1190 | 930 | 9 | 1011 | 14 | 530 | 676 | 510 | 890 | 250 | 4219 | 5906 | yes | CR |
| 64 | AU | 1100 | 1360 | 1.2 | 1170 | 990 | 9 | 1031 | 11 | 570 | 635 | 440 | 900 | 290 | 4265 | 5931 | yes | CR |
| 65 | AV | 1129 | 1250 | 1.6 | 1160 | 920 | 6 | 809 | 15 | 620 | 747 | 550 | 890 | 270 | 4274 | 5830 | yes | CR |
| 66 | AW | 1119 | 1290 | 1.8 | 1140 | 960 | 8 | 948 | 15 | 510 | 682 | 560 | 890 | 310 | 4333 | 5963 | yes | CR |
| 67 | AX | 1575 | 1580 | 2.0 | 1190 | 910 | 7 | 887 | 15 | 540 | 700 | 550 | 870 | 260 | 4184 | 5771 | yes | CR |
| 68 | AY | 1124 | 1240 | 1.8 | 1100 | 910 | 7 | 849 | 16 | 570 | 735 | 450 | 900 | 250 | 4214 | 5798 | yes | CR |
| 69 | AZ | 1043 | 1230 | 1.9 | 1100 | 980 | 5 | 727 | 10 | 600 | 625 | 600 | 910 | 280 | 4394 | 5746 | yes | CR |
| 70 | E | 1205 | 1290 | 1.7 | 1140 | 930 | 6 | 805 | 9 | 520 | 558 | 560 | 920 | 290 | 4423 | 5786 | no | GA |

| | | | | | | | | | | | | | | | | | | |
|---|---|---|---|---|---|---|---|---|---|---|---|---|---|---|---|---|---|---|
| * HR: hot-rolled steel sheet (no coating), CR: cold-rolled steel sheet (no coating), GI: hot-dip galvanized steel sheet (no alloying of galvanized coating), GA: galvannealed steel sheet The underlines indicate that the values are outside the scope of the present invention. | | | | | | | | | | | | | | | | | | |

**[Table 3-1]**

| | | Steel sheet microstructure | | | | | | | | Steel sheet properties | | | LME evaluation test | | | |
|---|---|---|---|---|---|---|---|---|---|---|---|---|---|---|---|---|
| Steel sheet sample No. | Steel symbol | TM + B (%) | FM (%) | γR (%) | Balance (%) | Nbₛₒₗ (mass %) | Nbₚᵣₑ (mass %) | Formula1 | Amount of diffusible hydrogen (mass ppm) | TS (MPa) | EI (%) | TS^{1.5} × EI (MPa·%) | Electrode inclination angle (°) | Holding time (s) | Evaluation results | Remarks |
| 1 | A | 72 | 1 | 14 | 13 | 0.002 | 0.004 | 0.50 | 0.02 | 1173 | 15.4 | 618682 | 3 | 0.12 | ⊚ | Inventive Ex. |
| 2 | A | 64 | 6 | 11 | 19 | 0.002 | 0.005 | 0.58 | 0.02 | 1180 | 12.7 | 514786 | 3 | 0.14 | ⊚ | Inventive Ex. |
| 3 | B | 84 | 4 | 9 | 3 | 0.002 | 0.007 | 0.45 | 0.03 | 1415 | 10.5 | 558887 | 5 | 0.08 | △ | Inventive Ex. |
| 4 | B | 58 | 16 | 10 | 16 | 0.003 | 0.008 | 0.55 | 0.02 | 1339 | 12.0 | 587966 | 3 | 0.14 | ⊚ | Inventive Ex. |
| 5 | C | 52 | 17 | 11 | 20 | 0.002 | 0.007 | 0.47 | 0.04 | 1453 | 8.5 | 470779 | 3 | 0.10 | ⊚ | Inventive Ex. |
| 6 | C | 59 | 14 | 9 | 18 | 0.002 | 0.007 | 0.47 | 0.01 | 1414 | 11.0 | 584880 | 4 | 0.10 | ○ | Inventive Ex. |
| 7 | C | 76 | 15 | 9 | 0 | 0.002 | 0.007 | 0.47 | 0.14 | 1526 | 10.6 | 631884 | 5 | 0.14 | ○ | Inventive Ex. |
| 8 | C | 75 | 16 | 7 | 2 | 0.002 | 0.007 | 0.47 | 0.18 | 1512 | 8.2 | 482105 | 3 | 0.08 | △ | Inventive Ex. |
| 9 | C | 73 | 18 | 8 | 1 | 0.002 | 0.007 | 0.47 | 0.11 | 1498 | 8.9 | 516010 | 4 | 0.10 | △ | Inventive Ex. |
| 10 | D | 81 | 6 | 12 | 1 | 0.003 | 0.007 | 0.48 | 0.03 | 1563 | 12.1 | 747694 | 3 | 0.08 | ⊚ | Inventive Ex. |
| 11 | D | 66 | 19 | 9 | 6 | 0.003 | 0.008 | 0.52 | 0.03 | 1584 | 9.5 | 598903 | 5 | 0.12 | ⊚ | Inventive Ex. |
| 12 | D | 71 | 21 | 8 | 0 | 0.001 | 0.004 | 0.24 | 0.01 | 1540 | 8.2 | 495559 | 5 | 0.14 | × | Comp. Ex. |
| 13 | D | 65 | 18 | 11 | 6 | 0.002 | 0.006 | 0.38 | 0.02 | 1476 | 12.4 | 703155 | 5 | 0.14 | × | Comp. Ex. |
| 14 | D | 72 | 18 | 10 | 0 | 0.002 | 0.005 | 0.33 | 0.02 | 1571 | 10.0 | 622679 | 3 | 0.14 | × | Comp. Ex. |
| 15 | D | 71 | 19 | 7 | 3 | 0.002 | 0.005 | 0.33 | 0.02 | 1460 | 7.2 | 401663 | 5 | 0.08 | × | Comp. Ex. |
| 16 | D | 25 | 1 | 13 | 61 | 0.003 | 0.009 | 0.57 | 0.04 | 953 | 15.4 | 453065 | 3 | 0.10 | ⊚ | Comp. Ex. |
| 17 | D | 84 | 3 | 7 | 6 | 0.002 | 0.005 | 0.33 | 0.03 | 1530 | 7.8 | 466801 | 4 | 0.12 | × | Comp. Ex. |
| 18 | D | 85 | 7 | 7 | 1 | 0.002 | 0.006 | 0.38 | 0.02 | 1484 | 7.6 | 434475 | 4 | 0.12 | × | Comp. Ex. |
| 19 | D | 83 | 5 | 6 | 6 | 0.002 | 0.004 | 0.29 | 0.04 | 1497 | 7.1 | 411236 | 4 | 0.12 | × | Comp. Ex. |
| 20 | D | 83 | 7 | 6 | 4 | 0.001 | 0.006 | 0.33 | 0.03 | 1499 | 6.9 | 400453 | 4 | 0.12 | × | Comp. Ex. |
| 21 | D | 69 | 17 | 7 | 7 | 0.004 | 0.009 | 0.62 | 0.04 | 1534 | 7.8 | 468633 | 4 | 0.14 | ⊚ | Inventive Ex. |
| 22 | E | 62 | 21 | 7 | 10 | 0.003 | 0.012 | 0.47 | 0.01 | 1785 | 12.0 | 904979 | 3 | 0.10 | ⊚ | Inventive Ex. |
| 23 | F | 84 | 8 | 6 | 2 | 0.004 | 0.009 | 0.51 | 0.01 | 1328 | 12.3 | 595254 | 4 | 0.10 | ⊚ | Inventive Ex. |
| 24 | G | 74 | 13 | 11 | 2 | 0.003 | 0.013 | 0.40 | 0.04 | 1456 | 13.0 | 722246 | 5 | 0.10 | ○ | Inventive Ex. |
| 25 | H | 67 | 4 | 12 | 17 | 0.003 | 0.010 | 0.56 | 0.04 | 1148 | 14.3 | 556223 | 3 | 0.12 | ⊚ | Inventive Ex. |
| 26 | I | 54 | 13 | 14 | 19 | 0.003 | 0.009 | 0.60 | 0.02 | 1581 | 8.1 | 509193 | 3 | 0.14 | ⊚ | Inventive Ex. |
| 27 | J | 60 | 24 | 9 | 7 | 0.001 | 0.002 | 0.41 | 0.04 | 1337 | 10.0 | 488874 | 4 | 0.10 | Δ | Inventive Ex. |
| 28 | K | 82 | 3 | 10 | 5 | 0.001 | 0.003 | 0.44 | 0.03 | 1352 | 10.9 | 541866 | 3 | 0.14 | ○ | Inventive Ex. |
| 29 | L | 81 | 7 | 11 | 1 | 0.005 | 0.011 | 0.55 | 0.04 | 1480 | 12.4 | 706016 | 4 | 0.10 | ⊚ | Inventive Ex. |
| 30 | M | 84 | 1 | 13 | 2 | 0.003 | 0.012 | 0.46 | 0.02 | 1014 | 14.8 | 477880 | 4 | 0.08 | ○ | Inventive Ex. |
| 31 | N | 84 | 4 | 8 | 4 | 0.002 | 0.006 | 0.55 | 0.05 | 1576 | 10.2 | 638167 | 3 | 0.12 | ⊚ | Inventive Ex. |
| 32 | Q | 83 | 0 | 7 | 10 | 0.005 | 0.012 | 0.57 | 0.04 | 946 | 8.3 | 241499 | 4 | 0.10 | ⊚ | Comp. Ex. |
| 33 | P | 75 | 15 | 8 | 2 | 0.003 | 0.007 | 0.47 | 0.02 | 1494 | 9.4 | 542817 | 4 | 0.14 | × | Comp. Ex. |
| 34 | Q | 84 | 2 | 5 | 9 | 0.004 | 0.012 | 0.58 | 0.03 | 1356 | 4.8 | 239679 | 4 | 0.10 | ⊚ | Comp. Ex. |
| 35 | R | 52 | 1 | 28 | 19 | 0.002 | 0.009 | 0.47 | 0.02 | 1012 | 28.4 | 914301 | 4 | 0.12 | × | Comp. Ex. |
| 36 | S | 34 | 1 | 12 | 53 | 0.002 | 0.006 | 0.50 | 0.01 | 974 | 14.9 | 452923 | 5 | 0.08 | ○ | Comp. Ex. |
| 37 | T | 64 | 28 | 6 | 2 | 0.002 | 0.007 | 0.44 | 0.01 | 1537 | 6.2 | 373596 | 4 | 0.08 | ○ | Comp. Ex. |
| 38 | U | 63 | 24 | 10 | 3 | 0.001 | 0.003 | 0.45 | 0.03 | 1392 | 11.0 | 571283 | 5 | 0.10 | × | Comp. Ex. |
| 39 | V | 80 | 3 | 9 | 8 | 0.002 | 0.004 | 0.50 | 0.02 | 1512 | 10.7 | 629088 | 5 | 0.12 | × | Comp. Ex. |
| 40 | W | 43 | 6 | 9 | 42 | 0.002 | 0.007 | 0.50 | 0.01 | 977 | 10.3 | 314542 | 5 | 0.14 | ⊚ | Comp. Ex. |
| 41 | X | 49 | 18 | 14 | 19 | 0.004 | 0.008 | 0.44 | 0.01 | 1259 | 17.6 | 786233 | 3 | 0.10 | × | Comp. Ex. |
| 42 | Y | 52 | 19 | 9 | 20 | 0.000 | 0.000 | - | 0.03 | 1308 | 9.1 | 430480 | 5 | 0.12 | × | Comp. Ex. |
| 43 | Z | 54 | 20 | 8 | 18 | 0.062 | 0.231 | 0.49 | 0.01 | 1504 | 9.5 | 554109 | 4 | 0.10 | × | Comp. Ex. |

The underlines indicate that the values are outside the scope of the present invention. TM: tempered martensite, B: bainite, FM: fresh martensite, γR: retained austenite In the LME evaluation test results, ⊚, ∘, and △ indicate excellent LME resistance, and × indicates poor LME resistance.

**[Table 3-2]**

| | | Steel sheet microstructure | | | | | | | | Steel sheet properties | | | LME evaluation test | | | |
|---|---|---|---|---|---|---|---|---|---|---|---|---|---|---|---|---|
| Steel sheet sample No. | Steel symbol | TM + B (%) | FM (%) | γR (%) | Balance (%) | Nbₛₒₗ (mass %) | Nbₚᵣₑ (mass %) | Formula1 | Amount of diffusible hydrogen (mass ppm) | TS (MPa) | El (%) | TS^{1.5} × El (MPa %) | Electrode inclination angle (°) | Holding time (s) | Evaluation results | Remarks |
| 44 | AA | 83 | 2 | 9 | 6 | 0.001 | 0.005 | 0.51 | 0.01 | 1527 | 8.2 | 489297 | 5 | 0.12 | ⊚ | Inventive Ex. |
| 45 | AB | 71 | 20 | 7 | 2 | 0.002 | 0.006 | 0.53 | 0.04 | 1522 | 10.8 | 641277 | 5 | 0.10 | ⊚ | Inventive Ex. |
| 46 | AC | 80 | 1 | 14 | 5 | 0.002 | 0.009 | 0.43 | 0.03 | 1124 | 16.2 | 610470 | 5 | 0.12 | Δ | Inventive Ex. |
| 47 | AD | 72 | 17 | 11 | 0 | 0.002 | 0.005 | 0.43 | 0.02 | 1178 | 12.3 | 497305 | 5 | 0.08 | Δ | Inventive Ex. |
| 48 | AE | 80 | 2 | 16 | 2 | 0.005 | 0.011 | 0.49 | 0.03 | 1118 | 18.8 | 702782 | 4 | 0.10 | ○ | Inventive Ex. |
| 49 | AF | 63 | 24 | 10 | 3 | 0.003 | 0.008 | 0.49 | 0.03 | 1308 | 9.4 | 444672 | 4 | 0.12 | ⊚ | Inventive Ex. |
| 50 | AG | 84 | 1 | 8 | 7 | 0.001 | 0.003 | 0.47 | 0.01 | 1292 | 9.1 | 422606 | 3 | 0.14 | Δ | Inventive Ex. |
| 51 | AH | 79 | 4 | 9 | 8 | 0.003 | 0.007 | 0.48 | 0.01 | 1321 | 9.6 | 460920 | 3 | 0.12 | ⊚ | Inventive Ex. |
| 52 | AI | 80 | 3 | 17 | 0 | 0.003 | 0.007 | 0.46 | 0.04 | 1116 | 20.5 | 764276 | 4 | 0.12 | Δ | Inventive Ex. |
| 53 | AJ | 80 | 1 | 11 | 8 | 0.002 | 0.006 | 0.44 | 0.03 | 1261 | 11.7 | 523912 | 5 | 0.08 | ○ | Inventive Ex. |
| 54 | AK | 81 | 4 | 14 | 1 | 0.002 | 0.007 | 0.42 | 0.04 | 1152 | 13.3 | 520032 | 3 | 0.08 | ○ | Inventive Ex. |
| 55 | AL | 79 | 4 | 15 | 2 | 0.003 | 0.008 | 0.42 | 0.02 | 1090 | 18.8 | 676546 | 3 | 0.12 | Δ | Inventive Ex. |
| 56 | AM | 77 | 2 | 13 | 8 | 0.001 | 0.005 | 0.43 | 0.03 | 1300 | 13.6 | 637461 | 3 | 0.12 | Δ | Inventive Ex. |
| 57 | AN | 79 | 6 | 12 | 3 | 0.002 | 0.006 | 0.49 | 0.03 | 1257 | 13.1 | 583814 | 4 | 0.08 | ⊚ | Inventive Ex. |
| 58 | AO | 71 | 16 | 11 | 2 | 0.003 | 0.009 | 0.41 | 0.03 | 1130 | 12.5 | 474819 | 3 | 0.10 | ○ | Inventive Ex. |
| 59 | AP | 47 | 24 | 10 | 19 | 0.003 | 0.009 | 0.47 | 0.04 | 1265 | 11.8 | 530906 | 4 | 0.10 | ○ | Inventive Ex. |
| 60 | AQ | 52 | 20 | 10 | 18 | 0.003 | 0.008 | 0.41 | 0.02 | 1112 | 12.4 | 459810 | 4 | 0.14 | ⊚ | Inventive Ex. |
| 61 | AR | 83 | 1 | 12 | 4 | 0.004 | 0.009 | 0.46 | 0.02 | 1087 | 14.0 | 501733 | 3 | 0.12 | ⊚ | Inventive Ex. |
| 62 | AS | 80 | 8 | 6 | 6 | 0.002 | 0.010 | 0.46 | 0.02 | 1425 | 7.4 | 398065 | 5 | 0.12 | ○ | Inventive Ex. |
| 63 | AT | 64 | 24 | 8 | 4 | 0.003 | 0.008 | 0.55 | 0.02 | 1398 | 8.2 | 428622 | 3 | 0.08 | ⊚ | Inventive Ex. |
| 64 | AU | 57 | 25 | 7 | 11 | 0.004 | 0.010 | 0.88 | 0.03 | 1636 | 9.5 | 628635 | 5 | 0.10 | ○ | Inventive Ex. |
| 65 | AV | 59 | 24 | 12 | 5 | 0.005 | 0.006 | 0.42 | 0.05 | 1374 | 14.4 | 733403 | 3 | 0.08 | ⊚ | Inventive Ex. |
| 66 | AW | 68 | 17 | 9 | 6 | 0.005 | 0.009 | 0.54 | 0.02 | 1399 | 13.1 | 685485 | 5 | 0.10 | ○ | Inventive Ex. |
| 67 | AX | 61 | 22 | 5 | 12 | 0.092 | 0.101 | 0.41 | 0.05 | 1639 | 6.8 | 451209 | 4 | 0.12 | Δ | Inventive Ex. |
| 68 | AY | 66 | 18 | 9 | 7 | 0.005 | 0.010 | 0.63 | 0.04 | 1360 | 11.4 | 571759 | 4 | 0.08 | ○ | Inventive Ex. |
| 69 | AZ | 84 | 4 | 9 | 3 | 0.003 | 0.010 | 0.81 | 0.03 | 1502 | 10.9 | 634500 | 3 | 0.10 | ○ | Inventive Ex. |
| 70 | E | 63 | 22 | 6 | 9 | 0.003 | 0.013 | 0.84 | 0.46 | 1798 | 10.6 | 808147 | 5 | 0.10 | Δ | Inventive Ex. |

The underlines indicate that the values are outside the scope of the present invention. TM: tempered martensite, B: bainite, FM: fresh martensite, yR: retained austenite In the LME evaluation test results, ⊚, ∘, and △ indicate excellent LME resistance, and × indicates poor LME resistance.

The area fractions of fresh martensite, tempered martensite, and bainite were determined by the following method. A thickness-direction cross-section (L cross-section) of each steel sheet, which was parallel to the rolling direction of the sheet, was polished and then etched with Nital. The cross-section was observed by a scanning electron microscope (SEM) at 2000-fold magnification in 10 fields of view at a 1/4 thickness position (a position at a distance of 1/4 of the sheet thickness from the steel sheet surface). Using a microstructural image obtained, the area fractions of constituent microstructures (the total fraction of tempered martensite and bainite, and the fraction of fresh martensite) were calculated. In the microstructural image, fresh martensite was determined by a light gray microstructural region, and tempered martensite and bainite were determined by a dark gray region in which carbides were precipitated.

The area fraction of retained austenite was determined by the following method. Each steel sheet was polished from the 1/4 thickness position to a plane by a thickness of 0.1 mm, and then further chemically polished to a plane by a thickness of 0.1 mm. The plane (surface) was subjected to X-ray diffraction analysis using CoKα rays to measure the integrated intensity ratios of the diffraction peaks of the {200}, {220} and {311} planes of fcc iron, and the {200}, {211} and {220} planes of bcc iron. The nine integrated intensity ratios obtained were averaged to determine the area fraction of retained austenite.

The amount of hydrogen in steel was determined by the following method. Test specimens of about 5 × 30 mm were cut out from a hot-rolled steel sheet, a cold-rolled steel sheet, and a galvanized steel sheet. For the test specimen of galvanized steel sheet, the coating on the surface of the test specimen was removed in advance using a router (precision grinder). Each test specimen was placed in a quartz tube, and the internal atmosphere of the tube was replaced with Ar, and then heated at 200°C/hr. Hydrogen generated until the temperature reached 400°C was subjected to gas chromatography to measure the amount of released hydrogen by a temperature rise analysis method. The cumulative value of the amount of hydrogen detected in the temperature range from room temperature (25°C) to less than 250°C was taken as the amount of diffusible hydrogen.

The total amount of Nb contained in the steel (Nbₜₒₜₐₗ), the amount of dissolved Nb in the steel sheet (Nbₛₒₗ), and the amount of Nb in Nb precipitates having a particle size of less than 20 nm (Nbₚᵣₑ) were measured in the following manner. The total amount of Nb contained in the steel (Nb) was measured by wet chemical analysis. The amount of Nb in Nb precipitates having a particle size of 20 nm or less was measured by the following method. Precipitates in the steel material were captured as residues, and the amount of Nb in all residues was determined. Thereafter, the amount of Nb present in residues having a particle size of 20 nm or more was determined. The amount of Nb in Nb precipitates having a particle size of 20 nm or less was determined as the difference between the amount of Nb in all residues and the amount of Nb present in the residues having a particle size of 20 nm or more. Specific procedures are as follows. A plurality of test specimens of about 20 × 50 mm were cut out from a hot-rolled steel sheet, a cold-rolled steel sheet, or a galvanized steel sheet. For a test specimen of a galvanized steel sheet, the coating on the surface of the test specimen was removed in advance using a router (precision grinder). The surface of each test specimen was polished about 50 µm by preliminary electrolytic polishing to obtain a fresh surface. The resulting test specimen was subjected to electrolysis using 10 vol % acetylacetone - 1 mass % tetramethylammonium chloride - methanol as an electrolytic solution for extracting precipitates. The resulting electrolytic solution after electrolysis was passed through a filter having a pore size of 0.2 µm to capture residues. The residues were then decomposed with an acid, and the Nb concentration was quantified in mass % unit using ICP emission spectrometry. The value obtained was used as the amount of Nb in all residues. Subsequently, a remaining test specimen was subjected to electrolysis using 10 vol % acetylacetone - 1 mass % tetramethylammonium chloride - methanol. Thereafter, the residual portion of the metal sample, remaining after the electrolysis, was immersed in separately prepared methanol, and residues, etc. attached to the residual portion of the metal sample were collected in a container using ultrasonic vibration. Thereafter, the electrolytic solution after electrolysis and the methanol containing the residues that had been attached to the residual portion of the metal sample were passed through an alumina filter having a pore size of 20 nm to capture residues. The residues were immersed in hexametaphosphoric acid and dispersed in the hexametaphosphoric acid using ultrasonic vibration. The residues, dispersed in hexametaphosphoric acid, were supplemented using a new alumina filter having a pore size of 20 nm. The residues captured on the alumina filter had a particle size of 20 nm or more. The residues were decomposed with an acid, and the Nb concentration was quantified in mass % unit using ICP emission spectrometry. The value obtained was used as the amount of Nb present in the residues having a particle size of 20 nm or more. The difference between the amount of Nb in all residues and the amount of Nb present in the residues having a particle size of 20 nm or more was taken as the amount of Nb in Nb precipitates having a particle size of 20 nm or less (Nbₚᵣₑ). Further, the amount of dissolved Nb in the steel sheet (Nbₛₒₗ) was determined as the difference between the total amount of Nb contained in the steel (Nb) and the amount of Nb in all residues determined by the above method.

While the above-described Nb precipitates are composed mainly of NbC, an NbN precipitate or other Nb precipitates may be contained in the steel sheet.

A tensile test was performed according to JIS Z 2241 (2011) using a JIS No. 5 test specimen which had been taken from a steel sheet such that the tensile direction was perpendicular to the rolling direction of the steel sheet, and the TS (tensile strength) and EL (total elongation) of the test specimen were measured. In the Examples, steel sheets having a TS of 980 MPa or more were evaluated as acceptable, judging that the intended strength was achieved. Steel sheets having a "TS^{1.5} × El" of 390,000 or more were evaluated as acceptable, judging that the intended formability was achieved.

The LME resistance was evaluated in the following manner. A sample, having the dimensions of: 100 mm in a direction perpendicular to the rolling direction, and 30 mm in the rolling direction, was taken from a steel sheet. The sample and a 980GA sample having the same size were stacked to prepare an evaluation sample.

Resistance spot welding was performed on the evaluation sample under the conditions of an electrode inclination angle of θ and a welding pressure of 3.5 kN. The electrode inclination angle in spot welding is herein defined as the angle θ between a line passing through the major axis of a nugget and a line parallel to the surface of a steel sheet in a cross-section of a spot-welded member. The welding current pattern was controlled so that the diameter of a nugget formed would fall within the range of 3.5√t to 5.5√t, t being the thickness (1.2 mm) of one steel sheet. In the resistance spot welding, Dr6-type CuCr electrodes were used, and the clearance between the evaluation sample and an electrode was 2.0 mm. The electrode inclination angles and holding times in the LME resistance evaluation tests are shown in Tables 3-1 and 3-2.

In each evaluation test, 5 evaluation samples were spot-welded to produce welded members, and a cross-section of each spot-welded member was observed using an optical microscope (100-fold magnification) to evaluate the LME resistance. When the number of members with cracking was two or less, and the average cracking depth was less than 100 µm (including no occurrence of cracking), the steel sheet was rated "⊚", when the number of members with cracking was two or less, and the average cracking depth was not less than 100 µm and not more than 300 µm, the steel sheet was rated "∘", when the number of members with cracking was two or less, and the average cracking depth was 300 µm or more, the steel sheet was rated "△", and when the number of members with cracking was three or more, the steel sheet was rated "×". In the Examples, the steel sheets rated ⊚, ∘, and △ were judged to have excellent LME resistance and referred to as Inventive Examples, while the steel sheets rated × were judged to have poor LME resistance and referred to as Comparative Examples.

The high-strength steel sheets of the Inventive Examples all have a high TS and a good TS × El balance, and are excellent in LME resistance, whereas the steel sheets of the Comparative Examples are poor in at least one of TS, TS × El balance, and LME resistance.

## Claims

1. A high-strength steel sheet having a chemical composition comprising, in mass %:
C: not less than 0.030% and not more than 0.500%,
Si: more than 0.01% and not more than 2.50%,
Mn: not less than 0.10% and not more than 5.00%,
P: 0.100% or less,
S: 0.0200% or less,
Al: 0.100% or less,
N: 0.0100% or less,
O: 0.0100% or less,
Ti: not less than 0.010% and not more than 0.200%, and
Nb: not less than 0.005% and not more than 0.500%,
with the balance being Fe and incidental impurities,
wherein in the microstructure of the steel sheet at a 1/4 thickness position,
the total area fraction of tempered martensite and bainite is not less than 40% and not more than 85%,
the area fraction of fresh martensite is not less than 0% and not more than 25%,
the area fraction of retained austenite is not less than 5% and not more than 20%, and
the balance includes at least one of ferrite and pearlite at an area fraction of not less than 0% and not more than 20%,
wherein the relationship between the amount of dissolved Nb (Nbₛₒₗ), the amount of Nb in Nb precipitates having a particle size of less than 20 nm (Nbₚᵣₑ), and the total amount of Nb contained in the steel sheet (Nb) satisfies the following Formula 1, and
wherein the amount of diffusible hydrogen in the steel is 0.50 mass ppm or less: $\left({Nb}_{sol}/Nb\right) + \left({Nb}_{pre}/Nb\right) \geq 0.40$ where Nbₛₒₗ represents the amount (mass %) of dissolved Nb, and Nbₚᵣₑ represents the amount (mass %) of Nb in Nb precipitates having a particle size of less than 20 nm.

2. The high-strength steel sheet according to claim 1, wherein the chemical composition further comprises, in mass %, one or two or more selected from the following:
V: 0.500% or less,
Ta: 0.10% or less,
W: 0.10% or less,
B: 0.0100% or less,
Cr: 1.00% or less,
Mo: 1.00% or less,
Co: 1.00% or less,
Ni: 1.00% or less,
Cu: 1.00% or less,
Sn: 0.200% or less,
Sb: 0.200% or less,
Ca: 0.0100% or less,
Mg: 0.0100% or less,
REM: 0.0100% or less,
Zr: 0.100% or less,
Te: 0.100% or less,
Hf: 0.10% or less, and
Bi: 0.200% or less.

3. The high-strength steel sheet according to claim 1 or 2, having a coating layer on the surface of the steel sheet.

4. The high-strength steel sheet according to claim 3, wherein the coating layer is an alloyed coating layer.

5. A method for manufacturing the high-strength steel sheet according to claim 1 or 2, comprising:
a slab heating step of heating a steel material having the chemical composition at a temperature equal to or higher than Tₛₒₗ°C represented by the following Formula 2 for 1.0 hours or more;
a hot rolling step;
a coiling step at a coiling temperature T_{CT}°C of 650°C or lower; and
an annealing step of heating a steel sheet to a soaking temperature T_{AT}°C, holding the steel sheet at the soaking temperature T_{AT}°C of not less than 750°C and not more than 950°C, and then cooling the steel sheet,
wherein Q_{HR} defined by Formula 3 in terms of a finish rolling start temperature T_{FET}°C, a finish rolling delivery temperature T_{FDT}°C, and an effective time t_{HR} from the start of finish rolling to the end of finish rolling in the hot rolling step,
Q_{CT} defined by Formula 4 in terms of a residence time t_{CT} from T_{FDT}°C to 650°C and the coiling temperature T_{CT}°C in the coiling step, and
Q_{AT} defined by Formula 5 in terms of the soaking temperature T_{AT}°C, a heating time t from 650°C to the soaking temperature T_{AT}°C, and a holding time t_{AT} at the soaking temperature T_{AT}°C in the annealing step, satisfy Formula 6: ${T}_{sol} = 7900 / \left(3.42-\left(log\left(\left[Nb%\right]\left[C%\right]\right)\right)\right) - 273$ where [Nb%] and [C%] respectively represent the Nb content (mass %) and the C content (mass %) of the steel; ${Q}_{HR} = 0.5 \left({T}_{FET}+{T}_{FDT}\right) \times {log}_{10} \left({t}_{HR}\right) ;$ ${Q}_{CT} = 0.5 \left({T}_{CT}+650\right) \times {log}_{10} \left({t}_{CT}\right) ;$ QAT = 0.5(650 + TAT) × log10(t) + TAT × log10(tAT); and${Q}_{HR} + {Q}_{CT} + {Q}_{AT} \leq 6000 .$

6. The method for manufacturing a high-strength steel sheet according to claim 5, wherein the value of Q_{AT} is 4700 or less.

7. The method for manufacturing a high-strength steel sheet according to claim 5 or 6, wherein the steel sheet after the annealing step is subjected to a coating treatment.

8. The method for manufacturing a high-strength steel sheet according to claim 7, wherein the coating treatment is an alloying coating treatment.
